



US005580689A

# United States Patent [19]

Chen et al.

[11] Patent Number: 5,580,689

[45] Date of Patent: Dec. 3, 1996

## [54] MIGRATION IMAGING MEMBERS

[75] Inventors: **Allan K. Chen**, Oakville; **Arnold L. Pundsack**, Georgetown, both of Canada; **Enrique Levy**, Englewood, N.J.; **Eric R. Endrizzi**, North York, Canada; **Richard N. Edwards**, Mississauga, Canada; **Arthur Y. Jones**, Mississauga, Canada; **Edward G. Zwartz**, Mississauga, Canada

[73] Assignee: **Xerox Corporation**, Stamford, Conn.

[21] Appl. No.: **523,574**

[22] Filed: **Sep. 5, 1995**

**Related U.S. Application Data**

[63] Continuation-in-part of Ser. No. 353,461, Dec. 9, 1994.

[51] Int. Cl.<sup>6</sup> ..... **G03G 17/10**

[52] U.S. Cl. ..... **430/41**

[58] Field of Search ..... 430/41

## [56] References Cited

## U.S. PATENT DOCUMENTS

|           |         |                      |        |
|-----------|---------|----------------------|--------|
| 4,012,250 | 3/1977  | Gotte .....          | 430/41 |
| 4,536,457 | 8/1985  | Tam .....            | 430/41 |
| 4,536,458 | 8/1985  | Ng .....             | 430/41 |
| 4,970,130 | 11/1990 | Tam et al. .....     | 430/41 |
| 5,102,756 | 5/1992  | Vincett et al. ..... | 430/41 |
| 5,215,838 | 6/1993  | Tam et al. .....     | 430/41 |

Primary Examiner—John Goodrow

Attorney, Agent, or Firm—Judith L. Byorick

## [57] ABSTRACT

Disclosed is a migration imaging member comprising a substrate and a softenable layer, said softenable layer comprising a softenable material, a pigment predominantly sensitive to infrared or red light radiation, and a migration marking material predominantly sensitive to radiation at a wavelength other than that to which the infrared or red light radiation sensitive pigment is sensitive contained at least at or near the surface of the softenable layer spaced from the substrate.

23 Claims, 4 Drawing Sheets

**FIG. 1****FIG. 2**

**FIG. 3****FIG. 4**

**FIG. 5****FIG. 6**

**FIG. 7**

## MIGRATION IMAGING MEMBERS

This application is a continuation-in-part of copending application U.S. Ser. No. 08/353,461, filed Dec. 9, 1994, entitled "Improved Migration Imaging Members", the disclosure of which is totally incorporated herein by reference.

## BACKGROUND OF THE INVENTION

The present invention is directed to improved infrared or red light sensitive migration imaging members. One embodiment of the present invention is directed to a migration imaging member comprising a substrate and a softenable layer, said softenable layer comprising a softenable material, a pigment predominantly sensitive to infrared or red light radiation, and a migration marking material predominantly sensitive to radiation at a wavelength other than that to which the infrared or red light radiation sensitive pigment is sensitive contained at least at or near the surface of the softenable layer spaced from the substrate. Another embodiment of the present invention is directed to a migration imaging process which comprises the steps of (A) providing a migration imaging member comprising a substrate and a softenable layer, said softenable layer comprising a softenable material, a pigment predominantly sensitive to infrared or red light radiation, and a migration marking material predominantly sensitive to radiation at a wavelength other than that to which the infrared or red light radiation sensitive pigment is sensitive contained at least at or near the surface of the softenable layer spaced from the substrate; (B) uniformly charging the imaging member; (C) subsequent to step B, exposing the charged imaging member to infrared or red light radiation at a wavelength to which the infrared or red light radiation sensitive pigment is sensitive in an imagewise pattern, thereby forming an electrostatic latent image on the imaging member; (D) subsequent to step B, uniformly exposing the imaging member to activating radiation at a wavelength to which the migration marking material is sensitive; and (E) subsequent to steps C and D, causing the softenable material to soften, thereby enabling the migration marking material to migrate through the softenable material toward the substrate in an imagewise pattern.

Migration imaging systems capable of producing high quality images of high optical contrast density and high resolution have been developed. Such migration imaging systems are disclosed in, for example, U.S. Pat. No. 3,975,195 (Goffe), U.S. Pat. No. 3,909,262 (Goffe et al.), U.S. Pat. No. 4,536,457 (Tam), U.S. Pat. No. 4,536,458 (Ng), U.S. Pat. No. 4,013,462 (Goffe et al.), and "Migration Imaging Mechanisms, Exploitation, and Future Prospects of Unique Photographic Technologies, XDM and AMEN", P. S. Vincent, G. J. Kovacs, M. C. Tam, A. L. Pundsack, and P. H. Soden, *Journal of Imaging Science* 30 (4) July/August, pp. 183-191 (1986), the disclosures of each of which are totally incorporated herein by reference. Migration imaging members containing charge transport materials in the softenable layer are also known, and are disclosed, for example, in U.S. Pat. No. 4,536,457 (Tam) and U.S. Pat. No. 4,536,458 (Ng). In a typical embodiment of these migration imaging systems, a migration imaging member comprising a substrate, a layer of softenable material, and photosensitive marking material is imaged by first forming a latent image by electrically charging the member and exposing the charged member to a pattern of activating electromagnetic radiation such as light. Where the photosensitive marking material is originally in the form of a fracturable layer contiguous with

the upper surface of the softenable layer, the marking particles in the exposed area of the member migrate in depth toward the substrate when the member is developed by softening the softenable layer.

The expression "softenable" as used herein is intended to mean any material which can be rendered more permeable, thereby enabling particles to migrate through its bulk. Conventionally, changing the permeability of such material or reducing its resistance to migration of migration marking material is accomplished by dissolving, swelling, melting, or softening, by techniques, for example, such as contacting with heat, vapors, partial solvents, solvent vapors, solvents, and combinations thereof, or by otherwise reducing the viscosity of the softenable material by any suitable means.

The expression "fracturable" layer or material as used herein means any layer or material which is capable of breaking up during development, thereby permitting portions of the layer to migrate toward the substrate or to be otherwise removed. The fracturable layer is preferably particulate in the various embodiments of the migration imaging members. Such fracturable layers of marking material are typically contiguous to the surface of the softenable layer spaced apart from the substrate, and such fracturable layers can be substantially or wholly embedded in the softenable layer in various embodiments of the imaging members.

The expression "contiguous" as used herein is intended to mean in actual contact, touching, also, near, though not in contact, and adjoining, and is intended to describe generically the relationship of the fracturable layer of marking material in the softenable layer with the surface of the softenable layer spaced apart from the substrate.

The expression "optically sign-retained" as used herein is intended to mean that the dark (higher optical density) and light (lower optical density) areas of the visible image formed on the migration imaging member correspond to the dark and light areas of the illuminating electromagnetic radiation pattern.

The expression "optically sign-reversed" as used herein is intended to mean that the dark areas of the image formed on the migration imaging member correspond to the light areas of the illuminating electromagnetic radiation pattern and the light areas of the image formed on the migration imaging member correspond to the dark areas of the illuminating electromagnetic radiation pattern.

The expression "optical contrast density" as used herein is intended to mean the difference between maximum optical density ( $D_{max}$ ) and minimum optical density ( $D_{min}$ ) of an image. Optical density is measured for the purpose of this invention by diffuse densitometers with a blue Wratten No. 47 filter. The expression "optical density" as used herein is intended to mean "transmission optical density" and is represented by the formula:

$$D = \log_{10}[I_o/I]$$

where  $I$  is the transmitted light intensity and  $I_o$  is the incident light intensity. For the purpose of this invention, all values of transmission optical density given in this invention include the substrate density of about 0.2 which is the typical density of a metallized polyester substrate.

There are various other systems for forming such images, wherein non-photosensitive or inert marking materials are arranged in the aforementioned fracturable layers, or dispersed throughout the softenable layer, as described in the aforementioned patents, which also disclose a variety of methods which can be used to form latent images upon migration imaging members.

Various means for developing the latent images can be used for migration imaging systems. These development methods include solvent wash away, solvent vapor softening, heat softening, and combinations of these methods, as well as any other method which changes the resistance of the softenable material to the migration of particulate marking material through the softenable layer to allow imagewise migration of the particles in depth toward the substrate. In the solvent wash away or meniscus development method, the migration marking material in the light struck region migrates toward the substrate through the softenable layer, which is softened and dissolved, and repacks into a more or less monolayer configuration. In migration imaging films supported by transparent substrates alone, this region exhibits a maximum optical density which can be as high as the initial optical density of the unprocessed film. On the other hand, the migration marking material in the unexposed region is substantially washed away and this region exhibits a minimum optical density which is essentially the optical density of the substrate alone. Therefore, the image sense of the developed image is optically sign reversed. Various methods and materials and combinations thereof have previously been used to fix such unfixed migration images. One method is to overcoat the image with a transparent abrasion resistant polymer by solution coating techniques. In the heat or vapor softening developing modes, the migration marking material in the light struck region disperses in the depth of the softenable layer after development and this region exhibits  $D_{min}$  which is typically in the range of 0.6 to 0.7. This relatively high  $D_{min}$  is a direct consequence of the depthwise dispersion of the otherwise unchanged migration marking material. On the other hand, the migration marking material in the unexposed region does not migrate and substantially remains in the original configuration, i.e. a monolayer. In known migration imaging films supported by transparent substrates, this region exhibits a maximum optical density ( $D_{max}$ ) of about 1.8 to 1.9. Therefore, the image sense of the heat or vapor developed images is optically sign-retained.

Techniques have been devised to permit optically sign-reversed imaging with vapor development, but these techniques are generally complex and require critically controlled processing conditions. An example of such techniques can be found in U.S. Pat. No. 3,795,512, the disclosure of which is totally incorporated herein by reference.

For many imaging applications, it is desirable to produce negative images from a positive original or positive images from a negative original (optically sign-reversing imaging), preferably with low minimum optical density. Although the meniscus or solvent wash away development method produces optically sign-reversed images with low minimum optical density, it entails removal of materials from the migration imaging member, leaving the migration image largely or totally unprotected from abrasion. Although various methods and materials have previously been used to overcoat such unfixed migration images, the post-development overcoating step can be impractically costly and inconvenient for the end users. Additionally, disposal of the effluents washed from the migration imaging member during development can also be very costly.

The background portions of an imaged member can sometimes be transparentized by means of an agglomeration and coalescence effect. In this system, an imaging member comprising a softenable layer containing a fracturable layer of electrically photosensitive migration marking material is imaged in one process mode by electrostatically charging the member, exposing the member to an imagewise pattern

of activating electromagnetic radiation, and softening the softenable layer by exposure for a few seconds to a solvent vapor thereby causing a selective migration in depth of the migration material in the softenable layer in the areas which were previously exposed to the activating radiation. The vapor developed image is then subjected to a heating step. Since the exposed particles gain a substantial net charge (typically 85 to 90 percent of the deposited surface charge) as a result of light exposure, they migrate substantially in depth in the softenable layer towards the substrate when exposed to a solvent vapor, thus causing a drastic reduction in optical density. The optical density in this region is typically in the region of 0.7 to 0.9 (including the substrate density of about 0.2) after vapor exposure, compared with an initial value of 1.8 to 1.9 (including the substrate density of about 0.2). In the unexposed region, the surface charge becomes discharged due to vapor exposure. The subsequent heating step causes the unmigrated, uncharged migration material in unexposed areas to agglomerate or flocculate, often accompanied by coalescence of the marking material particles, thereby resulting in a migration image of very low minimum optical density (in the unexposed areas) in the 0.25 to 0.35 range. Thus, the contrast density of the final image is typically in the range of 0.35 to 0.65. Alternatively, the migration image can be formed by heat followed by exposure to solvent vapors and a second heating step which also results in a migration image with very low minimum optical density. In this imaging system as well as in the previously described heat or vapor development techniques, the softenable layer remains substantially intact after development, with the image being self-fixed because the marking material particles are trapped within the softenable layer.

The word "agglomeration" as used herein is defined as the coming together and adhering of previously substantially separate particles, without the loss of identity of the particles.

The word "coalescence" as used herein is defined as the fusing together of such particles into larger units, usually accompanied by a change of shape of the coalesced particles towards a shape of lower energy, such as a sphere.

Generally, the softenable layer of migration imaging members is characterized by sensitivity to abrasion and foreign contaminants. Since a fracturable layer is located at or close to the surface of the softenable layer, abrasion can readily remove some of the fracturable layer during either manufacturing or use of the imaging member and adversely affect the final image. Foreign contamination such as finger prints can also cause defects to appear in any final image. Moreover, the softenable layer tends to cause blocking of migration imaging members when multiple members are stacked or when the migration imaging material is wound into rolls for storage or transportation. Blocking is the adhesion of adjacent objects to each other. Blocking usually results in damage to the objects when they are separated.

The sensitivity to abrasion and foreign contaminants can be reduced by forming an overcoating such as the overcoatings described in U.S. Pat. No. 3,909,262, the disclosure of which is totally incorporated herein by reference. However, because the migration imaging mechanisms for each development method are different and because they depend critically on the electrical properties of the surface of the softenable layer and on the complex interplay of the various electrical processes involving charge injection from the surface, charge transport through the softenable layer, charge capture by the photosensitive particles and charge ejection from the photosensitive particles, and the like, application of an overcoat to the softenable layer can cause

changes in the delicate balance of these processes and result in degraded photographic characteristics compared with the non-overcoated migration imaging member. Notably, the photographic contrast density can degraded.

U.S. Pat. No. 4,536,458 (Ng), the disclosure of which is totally incorporated herein by reference, discloses a migration imaging member comprising a substrate and an electrically insulating softenable layer on the substrate, the softenable layer comprising migration marking material located at least at or near the surface of the softenable layer spaced from the substrate, and a charge transport molecule. The migration imaging member is electrostatically charged, exposed to activating radiation in an imagewise pattern, and developed by decreasing the resistance to migration, by exposure either to solvent vapor or heat, of marking material in depth in the softenable layer at least sufficient to allow migration of marking material whereby marking material migrates toward the substrate in image configuration. The preferred thickness of the softenable layer is about 0.7 to 2.5 microns, although thinner and thicker layers can also be utilized.

U.S. Pat. No. 4,536,457 (Tam), the disclosure of which is totally incorporated herein by reference, discloses a process in which a migration imaging member comprising a substrate and an electrically insulating softenable layer on the substrate, the softenable layer comprising migration marking material located at least at or near the surface of the softenable layer spaced from the substrate, and a charge transport molecule (e.g. the imaging member described in U.S. Pat. No. 4,536,458) is uniformly charged and exposed to activating radiation in an imagewise pattern. The resistance to migration of marking material in the softenable layer is thereafter decreased sufficiently by the application of solvent vapor to allow the light exposed particles to retain a slight net charge to prevent agglomeration and coalescence and to allow slight migration in depth of marking material towards the substrate in image configuration, and the resistance to migration of marking material in the softenable layer is further decreased sufficiently by heating to allow non-exposed marking material to agglomerate and coalesce. The preferred thickness is about 0.5 to 2.5 microns, although thinner and thicker layers can be utilized.

U.S. Pat. No. 4,970,130 (Tam et al.), the disclosure of which is totally incorporated herein by reference, discloses a xeroprinting process which comprises (1) providing a xeroprinting master comprising (a) a substrate and (b) a softenable layer comprising a softenable material, a charge transport material capable of transporting charges of one polarity and migration marking material situated contiguous to the surface of the softenable layer spaced from the substrate, wherein a portion of the migration marking material has migrated through the softenable layer toward the substrate in imagewise fashion; (2) uniformly charging the xeroprinting master to a polarity opposite to the polarity of the charges that the charge transport material in the softenable layer is capable of transporting; (3) uniformly exposing the charged master to activating radiation, thereby discharging those areas of the master wherein the migration marking material has migrated toward the substrate and forming an electrostatic latent image; (4) developing the electrostatic latent image; and (5) transferring the developed image to a receiver sheet. The process results in greatly enhanced contrast potentials or contrast voltages between the charged and uncharged areas of the master subsequent to exposure to activating radiation, and the charged master can be developed with either liquid developers or dry developers. The contrast voltage of the electrostatic latent image obtainable

from this process generally initially increases with increasing flood exposure light intensity, typically reaches a plateau value of about 90 percent of the initially applied voltage even with further increase in flood exposure light intensity.

U.S. Pat. No. 5,215,838 (Tam et al.), the disclosure of which is totally incorporated herein by reference, discloses a migration imaging member comprising a substrate, an infrared or red light radiation sensitive layer comprising a pigment predominantly sensitive to infrared or red light radiation, and a softenable layer comprising a softenable material, a charge transport material, and migration marking material predominantly sensitive to radiation at a wavelength other than that to which the infrared or red light radiation sensitive pigment is sensitive contained at or near the surface of the softenable layer. When the migration imaging member is imaged and developed, it is particularly suitable for use as a xeroprinting master and can also be used for viewing or for storing data.

Migration imaging members are also suitable for other purposes, such as use as masks for exposing the photosensitive material in a printing plate for processes such as lithographic printing, and the like.

U.S. Pat. No. 5,102,756 (Vincett et al.), the disclosure of which is totally incorporated herein by reference, discloses a printing plate precursor which comprises a base layer, a layer of photohardenable material, and a layer of softenable material containing photosensitive migration marking material. Alternatively, the precursor can comprise a base layer and a layer of softenable photohardenable material containing photosensitive migration marking material. Also disclosed are processes for preparing printing plates from the disclosed precursors.

Copending application U.S. Ser. No. 08/353,461, entitled "Improved Migration Imaging Members", filed Dec. 9, 1994 with the named inventors Edward G. Zwart, Carol A. Jennings, Man C. Tam, Philip H. Soden, Arthur Y. Jones, Arnold L. Pundsack, Enrique Levy, Ah-Me Hor, William W. Limburg, John F. Yanus, Damodar M. Pal, and Dale S. Renfer, the disclosure of which is totally incorporated herein by reference, discloses migration imaging member comprising a substrate, a first softenable layer comprising a first softenable material and a first migration marking material contained at or near the surface of the first softenable layer spaced from the substrate, and a second softenable layer comprising a second softenable material and a second migration marking material. Also disclosed is a migration imaging process employing the aforesaid imaging member.

Copending application U.S. Ser. No. 08/413,667, entitled "Improved Apparatus and Process for Preparation of Migration Imaging Members", filed Mar. 30, 1995 with the named inventors Philip H. Soden and Arnold L. Pundsack, the disclosure of which is totally incorporated herein by reference, discloses an apparatus for evaporation of a vacuum evaporatable material onto a substrate, said apparatus comprising (a) a walled container for the vacuum evaporatable material having a plurality of apertures in a surface thereof, said apertures being configured so that the vacuum evaporatable material is uniformly deposited onto the substrate; and (b) a source of heat sufficient to effect evaporation of the vacuum evaporatable material from the container through the apertures onto the substrate, wherein the surface of the container having the plurality of apertures therein is maintained at a temperature equal to or greater than the temperature of the vacuum evaporatable material.

Copending application U.S. Ser. No. 08/432,401, entitled "Pre-Sensitized Infrared or Red Light Sensitive Migration Imaging Members", filed May 1, 1995 with the named

inventor Man C. Tam, the disclosure of which is totally incorporated herein by reference, discloses a process which comprises (1) providing a migration imaging member comprising a substrate, an infrared or red light radiation sensitive layer comprising a pigment predominantly sensitive to infrared or red light radiation, and a softenable layer comprising a softenable material, a charge transport material, and migration marking material predominantly sensitive to radiation at a wavelength other than that to which the infrared or red light sensitive pigment is predominantly sensitive contained at or near the surface of the softenable layer, said infrared or red light radiation sensitive layer being situated between the substrate and the softenable layer; (2) uniformly charging the imaging member; (3) subsequent to step (2), uniformly exposing the imaging member to activating radiation at a wavelength to which the migration marking material is sensitive; (4) subsequent to step (3), neutralizing charge on the surface of the imaging member spaced from the substrate, (5) subsequent to step (4), exposing the imaging member to infrared or red light radiation at a wavelength to which the infrared or red light radiation sensitive pigment is sensitive in an imagewise pattern, thereby forming an electrostatic latent image on the imaging member, wherein step (5) takes place at least 2 hours after completion of step (4); (6) subsequent to step (5), causing the softenable material to soften, thereby enabling the migration marking material to migrate through the softenable material toward the substrate in an imagewise pattern.

Copending application U.S. Ser. No. 08/432,291, entitled "Improved Migration Imaging Process", filed May 1, 1995 with the named inventors Man C. Tam and Edward G. Zwartz, the disclosure of which is totally incorporated herein by reference, discloses a process which comprises (a) providing a migration imaging member comprising (1) a substrate, (2) an infrared or red light radiation sensitive layer comprising a pigment predominantly sensitive to infrared or red light radiation, and (3) a softenable layer comprising a softenable material, a charge transport material, and a photosensitive migration marking material predominantly sensitive to radiation at a wavelength other than that to which the infrared or red light sensitive pigment is predominantly sensitive; (b) uniformly charging the imaging member; (c) subsequent to step (b), uniformly exposing the charged imaging member to a source of activating radiation with a wavelength to which the migration marking material is sensitive, wherein a filter comprising the infrared or red light radiation sensitive pigment is situated between the radiation source and the imaging member; (d) subsequent to step (b), exposing the imaging member to infrared or red light radiation at a wavelength to which the infrared or red light radiation sensitive pigment is sensitive in an imagewise pattern, thereby forming an electrostatic latent image on the imaging member; and (e) subsequent to steps (c) and (d), causing the softenable material to soften, thereby enabling the migration marking material to migrate through the softenable material toward the substrate in an imagewise pattern.

Copending application U.S. Ser. No. 08/432,448, entitled "Improved Overcoated Migration Imaging Members", filed May 1, 1995 with the named inventors Shadi L. Malhotra and Arthur Y. Jones, the disclosure of which is totally incorporated herein by reference, discloses a migration imaging member comprising (1) a substrate, (2) a softenable layer situated on the substrate, said softenable layer comprising a softenable material and a photosensitive migration marking material, and (3) an overcoating layer situated on the surface of the softenable layer spaced from the substrate,

said overcoating layer comprising a material selected from the group consisting of: (a) polyacrylic acids, (b) poly(hydroxyalkyl methacrylates), (c) poly(hydroxyalkylacrylates), (d) vinyl alcohol-vinyl acetate copolymers, (e) vinyl alcohol-vinyl butyral copolymers, (f) alkyl celluloses, (g) aryl celluloses, (h) hydroxyalkyl cellulose acrylates, (i) hydroxyaryl cellulose acrylates, (j) hydroxyalkyl cellulose methacrylates, (k) hydroxyaryl cellulose methacrylates, (l) cellulose-acrylamide adducts, (m) poly(vinyl butyral), (n) cyanoethylated celluloses, (o) cellulose acetate hydrogen phthalates, (p) hydroxypropylmethyl cellulose phthalates, (q) hydroxypropyl methyl cellulose succinates, (r) cellulose triacetates, (s) vinyl pyrrolidone-vinyl acetate copolymers, (t) vinyl chloride-vinylacetate-vinyl alcohol terpolymers, (u) ethylene-maleic anhydride copolymers, (v) styrene-maleic anhydride copolymers, (w) styrene-allyl alcohol copolymers, (x) poly(4-vinylpyridines), (y) polyester latexes, (z) vinyl chloride latexes, (aa) ethylene-vinyl chloride copolymer emulsions, (bb) poly vinyl acetate homopolymer emulsions, (cc) carboxylated vinyl acetate emulsion resins, (dd) vinyl acetate copolymer latexes, (ee) ethylene-vinyl acetate copolymer emulsions, (ff) acrylic-vinyl acetate copolymer emulsions, (gg) vinyl acrylic terpolymer latexes, (hh) acrylic emulsion latexes, (ii) polystyrene latexes, (jj) styrene-butadiene latexes, (kk) butadiene-acrylonitrile latexes, (ll) butadiene-acrylonitrile-styrene terpolymer latexes, (mm) propylene-acrylic acid copolymers, (nn) propylene-ethylene-acrylic acid terpolymers, (oo) poly(vinyl methyl ketones), (pp) poly(trimethyl hexamethylene) terephthalamides, (qq) chlorinated polypropylenes, (rr) poly(hexamethylene sebacates), (ss) poly(ethylene succinates), (tt) poly(caprolactams), (uu) poly(hexamethylene adipamides), (vv) poly(hexamethylene nonaneamides), (ww) poly(hexamethylene sebacamides), (xx) poly(hexamethylene dodecane diamides), (yy) poly(undecanoamides), (zz) poly(lauryllactams), (aaa) ethylene-methacrylic acid ionomers, and (bbb) mixtures thereof.

Copending application U.S. Ser. No. 08/432,380, entitled "Improved Migration Imaging Members", filed May 1, 1995 with the named inventor Shadi L. Malhotra, the disclosure of which is totally incorporated herein by reference, discloses a migration imaging member comprising (a) a substrate, (b) a softenable layer situated on one surface of the substrate, said softenable layer comprising a softenable material and a photosensitive migration marking material, and (c) an anti-static layer situated on the surface of the substrate opposite to the surface in contact with the softenable layer.

Copending application U.S. Ser. No. 08/442,227, entitled "Improved Migration Imaging Members", filed May 15, 1995 with the named inventors Shadi L. Malhotra, Liqin Chen, and Marie-Eve Perron, the disclosure of which is totally incorporated herein by reference, discloses a migration imaging member comprising (a) a substrate, (b) a softenable layer comprising a softenable material and a photosensitive migration marking material, and (c) a transparentizing agent which transparentizes migration marking material in contact therewith contained in at least one layer of the migration imaging member. Also disclosed is a process which comprises (1) providing a migration imaging member comprising (a) a substrate, (b) a softenable layer comprising a softenable material and a photosensitive migration marking material, and (c) a transparentizing agent which transparentizes migration marking material in contact therewith contained in at least one layer of the migration imaging member; (2) uniformly charging the imaging member; (3) subsequent to step (2), exposing the charged imaging member to activating radiation at a wavelength to which

the migration marking material is sensitive; (4) subsequent to step (3), causing the softenable material to soften and enabling a first portion of the migration marking material to migrate through the softenable material toward the substrate in an imagewise pattern while a second portion of the migration marking material remains substantially unmigrated within the softenable layer, wherein subsequent to migration of the first portion of migration marking material, either (a) the first portion of migration marking material contacts the transparentizing agent and the second portion of migration marking material does not contact the transparentizing agent; or (b) the second portion of migration marking material contacts the transparentizing agent and the first portion of migration marking material does not contact the transparentizing agent.

Copending application U.S. Ser. No. 08/441,360, entitled "Method For Obtaining Improved Image Contrast In Migration Imaging Members", filed May 15, 1995 with the named inventors William W. Limburg, Joseph Mammino, George Liebermann, Clifford H. Griffiths, Michael M. Shahin, Shadi L. Malhotra, Liqin Chen, and Marie-Eve Perron, the disclosure of which is totally incorporated herein by reference, discloses a process which comprises (a) providing a migration imaging member comprising (1) a substrate and (2) a softenable layer comprising a softenable material and a photosensitive migration marking material present in the softenable layer as a monolayer of particles situated at or near the surface of the softenable layer spaced from the substrate; (b) uniformly charging the imaging member; (3) imagewise exposing the charged imaging member to activating radiation at a wavelength to which the migration marking material is sensitive; (d) subsequent to step (c), causing the softenable material to soften and enabling a first portion of the migration marking material to migrate through the softenable material toward the substrate in an imagewise pattern while a second portion of the migration marking material remains substantially unmigrated within the softenable layer; and (e) contacting the second portion of the migration marking material with a transparentizing agent which transparentizes migration marking material.

Copending application U.S. Ser. No. 08/432,747, entitled "Process and Apparatus for Manufacturing Migration Imaging Members", filed May 2, 1995 with the named inventors Hardy Sonnenberg, Arnold L. Pundsack, Man C. Tam, and Enrique Levy, the disclosure of which is totally incorporated herein by reference, discloses a process and apparatus for preparing migration imaging members. Two substrates with softenable layers applied to them travel through a vacuum chamber where they are simultaneously exposed to vapor deposition of the migration marking material. After the migration marking material is deposited, the two softenable layers are laminated together in the same vacuum chamber to form the migration imaging member. In one of the embodiments, the softenable layers are applied to the substrates in the same sweep of the substrate through the vacuum chamber vapor deposition and lamination steps.

Copending application U.S. Ser. No. 08/434,954, entitled "Film Loading Pins for External Drum Scanners", filed May 4, 1995 with the named inventors Robert J. Kleckner and Sandra Graveson, the disclosure of which is totally incorporated herein by reference, discloses a registration pin for a rotating drum recorder device which cooperates with a film to register and support the film during loading the film onto the drum. The registration pin has a reduced profile to reduce the overall size of the drum. The pin also has a construction to permit loading of different types of films onto the drum. The head of the registration pin is provided with a profile

that supports and positions the film on the drum, even though the registration pin is shorter than conventional pins. The registration pin includes at least one protrusion to sandwich the film against the surface of the drum. The protrusion may take any appropriate form. The protrusion may include a "teardrop" shaped form, in order to positively hold the film on the drum.

Copending application U.S. Ser. No. 08/434,962, entitled "Modular Charging Device for Imaging System", filed May 4, 1995 with the named inventors Robert J. Kleckner, Irena Makarchuk, and Frank Martines, the disclosure of which is totally incorporated herein by reference, discloses a modular charging device for use in a printing or imaging system which includes a plurality of individual charging units and means for arranging the plurality of individual charging units together in a modular fashion. The modular charging device may be arc-shaped to uniformly charge a rotating drum or a circular belt, or may be linear to uniformly charge a linear imaging member.

Copending application U.S. Ser. No. 08/434,960, entitled "Film Heat Processor and Method of Developing Digital Film", filed May 4, 1995 with the named inventors Abu S. Islam, Robert J. Kleckner, Leo Chin, Hardy Sonnenberg, and Anthony Klein, the disclosure of which is totally incorporated herein by reference, discloses an apparatus and method of developing a heat developing film which includes a film support surface for supporting a film and heaters for developing the film supported on the film support surface. The film support surface may either be stationary or form part of a film transport. The film transport may either be a continuous film transport or a reciprocating film transport. The continuous film transport may be inclined or include an input pinch roller. In addition, the heaters may either be stationary, reciprocatable, or pivotable. The heaters are radiant heaters which may include a profiled heater output to control distortion of the film. The apparatus may be provided as a stand-alone unit or may be coupled, either externally to or within, a film exposure device.

Copending application U.S. Ser. No. 08/434,961, entitled "A Device that Uses Radiant Heat to Desensitize Migration Imaging Film and Allow Daylight Film Handling", filed May 4, 1995 with the named inventors Irena Makarchuk, Sandra Graveson, Robert J. Kleckner, Leo Chin, and Abu S. Islam, the disclosure of which is totally incorporated herein by reference, discloses a heating device for desensitizing migration imaging film on an external imaging member scanner. The heating device is curved and has a large surface area to provide maximum heating efficiency. The heating device is mounted to a bracket connected to a scanner cartridge and moves integrally with the scanner cartridge in the direction of the longitudinal axis of the imaging member. The heating device heats the migration imaging film to a temperature to ensure that the surface charge on the film is changed, but is less than a temperature needed for selenium particle migration. As a result, the selenium in the migration imaging film is no longer sensitive under daylight conditions. Thus, the migration imaging film can be removed and heated under daylight conditions providing a significant advantage over film that must be removed and heated under red light conditions.

While known imaging members and imaging processes are suitable for their intended purposes, a need remains for improved migration imaging members. In addition, a need remains for infrared or red light sensitive migration imaging members which can be prepared or manufactured with improved cost effectiveness. Further, there is a need for infrared or red light sensitive migration imaging members

with improved resistance to scratching and other handling damage. Additionally, a need exists for infrared or red light sensitive migration imaging members wherein difficulties in applying an infrared or red light sensitive layer to the imaging member structure are reduced or eliminated. There is also a need for infrared or red light sensitive migration imaging members which, when imaged, exhibit improved optical density. In addition, there is a need for infrared or red light sensitive migration imaging members which exhibit improved uniformity of deposition of the infrared or red light sensitive material on the imaging member. Further, a need remains for infrared or red light sensitive imaging members wherein the need for a charge transport material in the softenable layer is reduced or eliminated. Additionally, a need remains for infrared or red light sensitive imaging members which exhibit reduced  $D_{min}$  values, particularly in the ultraviolet region. There is also a need for infrared or red light sensitive imaging members for which the required exposure times are reduced. A need further remains for infrared or red light sensitive imaging members which exhibit increased charge life prior to imaging. In addition, there is a need for infrared or red light sensitive imaging members which require lower concentrations of infrared or red light sensitive pigment, thereby enabling reduced cost.

#### SUMMARY OF THE INVENTION

It is an object of the present invention to provide migration imaging members with the above noted advantages.

It is another object of the present invention to provide improved migration imaging members.

It is yet another object of the present invention to provide infrared or red light sensitive migration imaging members which can be prepared or manufactured with improved cost effectiveness.

It is still another object of the present invention to provide infrared or red light sensitive migration imaging members with improved resistance to scratching and other handling damage.

Another object of the present invention is to provide infrared or red light sensitive migration imaging members wherein difficulties in applying an infrared or red light sensitive layer to the imaging member structure are reduced or eliminated.

Yet another object of the present invention is to provide infrared or red light sensitive migration imaging members which, when imaged, exhibit improved optical density.

Still another object of the present invention is to provide infrared or red light sensitive migration imaging members which exhibit improved uniformity of deposition of the infrared or red light sensitive material on the imaging member.

It is another object of the present invention to provide infrared or red light sensitive imaging members wherein the need for a charge transport material in the softenable layer is reduced or eliminated.

It is yet another object of the present invention to provide infrared or red light sensitive imaging members which exhibit reduced  $D_{min}$  values, particularly in the ultraviolet region.

It is still another object of the present invention to provide infrared or red light sensitive imaging members for which the required exposure times are reduced.

Another object of the present invention is to provide infrared or red light sensitive imaging members which

exhibit increased charge life prior to imaging. Yet another object of the present invention is to provide infrared or red light sensitive imaging members which require lower concentrations of infrared or red light sensitive pigment, thereby enabling reduced cost.

These and other objects of the present invention (or specific embodiments thereof) can be achieved by providing a migration imaging member comprising a substrate and a softenable layer, said softenable layer comprising a softenable material, a pigment predominantly sensitive to infrared or red light radiation, and a migration marking material predominantly sensitive to radiation at a wavelength other than that to which the infrared or red light radiation sensitive pigment is sensitive contained at least at or near the surface of the softenable layer spaced from the substrate. Another embodiment of the present invention is directed to a migration imaging process which comprises the steps of (A) providing a migration imaging member comprising a substrate and a softenable layer, said softenable layer comprising a softenable material, a pigment predominantly sensitive to infrared or red light radiation, and a migration marking material predominantly sensitive to radiation at a wavelength other than that to which the infrared or red light radiation sensitive pigment is sensitive contained at least at or near the surface of the softenable layer spaced from the substrate; (B) uniformly charging the imaging member; (C) subsequent to step B, exposing the charged imaging member to infrared or red light radiation at a wavelength to which the infrared or red light radiation sensitive pigment is sensitive in an imagewise pattern, thereby forming an electrostatic latent image on the imaging member; (D) subsequent to step B, uniformly exposing the imaging member to activating radiation at a wavelength to which the migration marking material is sensitive; and (E) subsequent to steps C and D, causing the softenable material to soften, thereby enabling the migration marking material to migrate through the softenable material toward the substrate in an imagewise pattern.

#### BRIEF DESCRIPTION OF THE DRAWINGS

FIG. 1 illustrates schematically a migration imaging member of the present invention.

FIGS. 2, 3, 4, 5, 6, and 7 illustrate schematically a process for imaging and developing migration imaging members of the present invention.

#### DETAILED DESCRIPTION OF THE INVENTION

The migration imaging member of the present invention comprises a substrate and a softenable layer. The softenable layer comprises a softenable material, a pigment predominantly sensitive to infrared or red light radiation, and a migration marking material predominantly sensitive to radiation at a wavelength other than that to which the infrared or red light radiation sensitive pigment is sensitive contained at or near the surface of the softenable layer spaced from the substrate.

As illustrated schematically in FIG. 1, migration imaging member 1 comprises in the order shown an optional anti-static layer 3 situated on a substrate 4, an optional adhesive layer 5 situated on substrate 4, an optional charge blocking layer 7 situated on optional adhesive layer 5, an optional charge transport layer 9 situated on optional charge blocking layer 7, a softenable layer 10 situated on optional charge transport layer 9, said softenable layer 10 comprising soft-

enable material 11, optional charge transport material 16, infrared or red light radiation sensitive pigment particles 14 dispersed within softenable material 11, and migration marking material 12 situated at or near the surface of softenable layer 10 spaced from substrate 4. Optional second softenable layer 18 is situated on first softenable layer 10 and comprises second softenable material 19, optional second charge transport material 20, and second migration marking material 21, shown in this embodiment situated at or near the surface of second softenable layer 18 in contact with softenable layer 10 (although second migration marking material 21 can be situated at or near the surface of second softenable layer 18 spaced from softenable layer 10, or can be distributed uniformly throughout second softenable layer 18, if desired). Optional overcoating layer 17 is situated on the surface of the imaging member spaced from substrate 4.

Any or all of the optional layers and materials shown in FIG. 1 can be absent from the imaging member. In addition, the optional layers present need not be in the order shown, but can be in any suitable arrangement. The migration imaging member can be in any suitable configuration, such as a web, a foil, a laminate, a strip, a sheet, a coil, a cylinder, a drum, an endless belt, an endless mobius strip, a circular disc, or any other suitable form.

The substrate can be either electrically conductive or electrically insulating. When conductive, the substrate can be opaque, translucent, semitransparent, or transparent, and can be of any suitable conductive material, including copper, brass, nickel, zinc, chromium, stainless steel, conductive plastics and rubbers, aluminum, semitransparent aluminum, steel, cadmium, silver, gold, paper rendered conductive by the inclusion of a suitable material therein or through conditioning in a humid atmosphere to ensure the presence of sufficient water content to render the material conductive, indium, tin, metal oxides, including tin oxide and indium tin oxide, and the like. When insulative, the substrate can be opaque, translucent, semitransparent, or transparent, and can be of any suitable insulative material, such as paper, glass, plastic, polyesters such as Mylar® (available from Du Pont) or Melinex® 442, (available from ICI Americas, Inc.), and the like. In addition, the substrate can comprise an insulative layer with a conductive coating, such as vacuum-deposited metallized plastic, such as titanized or aluminized Mylar® polyester, wherein the metallized surface is in contact with the softenable layer, a substrate such as polyester coated with another conductive material, such as a conductive oxide, including oxides of tin, indium, or the like, metallic microfibers in a polymer binder, copper iodide, or the like, or any other layer situated between the substrate and the softenable layer. The substrate has any effective thickness, typically from about 6 to about 250 microns, and preferably from about 50 to about 200 microns, although the thickness can be outside of this range.

The softenable layer can be of any suitable material, typically a plastic or thermoplastic material which is either heat softenable or soluble in a solvent or softenable, for example, in a solvent liquid, solvent vapor, heat, or any combinations thereof. When the softenable layer is to be softened or dissolved either during or after imaging, it should be soluble in a solvent that does not attack the migration marking material. By softenable is meant any material that can be rendered by a development step as described herein permeable to migration marking material migrating through its bulk. This permeability typically is achieved by a development step entailing dissolving, melting, or softening by contact with heat, vapors, partial solvents, as well as combinations thereof. Examples of suitable

softenable materials include styrene-acrylic copolymers, such as styrene-hexylmethacrylate copolymers, styrene acrylate copolymers, styrene butylmethacrylate copolymers, styrene butylacrylate ethylacrylate copolymers, styrene ethylacrylate acrylic acid copolymers, and the like, polystyrenes, including polyalphamethyl styrene, alkyd substituted polystyrenes, styrene-olefin copolymers, styrene-vinyltoluene copolymers, polyesters, polyurethanes, polycarbonates, polyterpenes, silicone elastomers, mixtures thereof, copolymers thereof, and the like, as well as any other suitable materials as disclosed, for example, in U.S. Pat. No. 3,975,195 and other U.S. patents directed to migration imaging members which have been incorporated herein by reference. The softenable layer can be of any effective thickness, typically from about 1 to about 30 microns, and preferably from about 2 to about 25 microns, although the thickness can be outside of this range.

The softenable layer also contains migration marking material. The migration marking material is electrically photosensitive or photoconductive, and is sensitive to radiation at a wavelength other than that to which the infrared or red light sensitive pigment is sensitive; while the migration marking material may exhibit some photosensitivity in the wavelength to which the infrared or red light sensitive pigment is sensitive, it is preferred that photosensitivity in this wavelength range be minimized so that the migration marking material and the infrared or red light sensitive pigment exhibit absorption peaks in distinct, different wavelength regions. The migration marking material preferably is particulate, wherein the particles are closely spaced from each other. Preferred migration marking materials generally are spherical in shape and submicron in size. The migration marking material generally is capable of substantial photodischarge upon electrostatic charging and exposure to activating radiation and is substantially absorbing and opaque to activating radiation in the spectral region where the photo-sensitive migration marking particles photogenerate charges. The migration marking material is preferably present in the softenable layer as a thin layer or monolayer of particles situated at or near the surface of the softenable layer spaced from the substrate, although the migration marking material may also be dispersed throughout the softenable layer. A monolayer of particles may be preferred because this configuration enables the highest possible  $D_{max}$  values for the lowest mass of migration marking material, and may also enable very low  $D_{min}$  values. In this embodiment, it is preferred that the monolayer of particles be situated in the softenable layer at or near the surface spaced from the substrate. When present as particles, the particles of migration marking material preferably have an average diameter of up to 2 microns, and more preferably of from about 0.1 micron to about 1 micron. Typically, the particles are situated at a distance of from about 0.01 micron to 0.1 micron from the softenable layer surface, although the distance can be outside this range. Preferably, the particles are situated at a distance of from about 0.005 micron to about 0.2 micron from each other, and more preferably at a distance of from about 0.05 micron to about 0.1 micron from each other, the distance being measured between the closest edges of the particles, i.e. from outer diameter to outer diameter. The migration marking material contiguous to the outer surface of the softenable layer is present in any effective amount, preferably from about 2 percent to about 25 percent by total weight of the softenable layer, and more preferably from about 5 to about 20 percent by total weight of the softenable layer.

Examples of suitable migration marking materials include selenium, alloys of selenium with alloying components such

as tellurium, arsenic, mixtures thereof, and the like, and any other suitable materials as disclosed, for example, in U.S. Pat. No. 3,975,195 and other U.S. patents directed to migration imaging members and incorporated herein by reference.

The migration marking particles can be included in the imaging members by any suitable technique. For example, a layer of migration marking particles can be placed at or just below the surface of a softenable layer by solution coating a substrate containing the softenable layer material, followed by heating the softenable material in a vacuum chamber to soften it, while at the same time thermally evaporating the migration marking material onto the softenable material in the vacuum chamber. Other techniques for preparing monolayers include cascade and electrophoretic deposition. An example of a suitable process for depositing migration marking material in the softenable layer is disclosed in U.S. Pat. No. 4,482,622, the disclosure of which is totally incorporated herein by reference.

The infrared or red light sensitive pigment is dispersed within the softenable material of the softenable layer. The infrared or red light sensitive pigment can be incorporated into the softenable layer by any suitable technique. For example, it can be mixed with the softenable material by dissolution in a common solvent. If desired, a mixture of solvents for the infrared or red light sensitive pigment and the softenable material can be employed to facilitate mixing and coating. In a preferred embodiment, the mixture is microfluidized or subjected to some other process suitable for reducing the pigment particle size such as ball milling, preferably followed by filtration of the solution. The softenable layer mixture can be applied to the substrate by any conventional process. Typical coating processes include draw bar coating, spray coating, extrusion, dip coating, gravure roll coating, wire-wound rod coating, air knife coating, reverse roll coating, slot die coating, and the like. The softenable material can be dispersed in a suitable solvent, followed by dispersing the pigment in the solution by ball milling, coating the dispersion onto the imaging member comprising the substrate and any previously coated layers, and evaporating the solvent to form a solid film. The softenable layer can also be applied by a lamination process.

Examples of suitable red light sensitive pigments include perylene pigments such as benzimidazole perylene, dibromoanthrathrone, crystalline trigonal selenium, beta-metal free phthalocyanine, azo pigments, and the like, as well as mixtures thereof. Examples of suitable infrared sensitive pigments include X-metal free phthalocyanine, metal phthalocyanines such as vanadyl phthalocyanine, chloroindium phthalocyanine, titanyl phthalocyanine, chloroaluminum phthalocyanine, copper phthalocyanine, magnesium phthalocyanine, and the like, squaraines, such as hydroxy squaraine, and the like as well as mixtures thereof. Examples of suitable optional polymeric binder materials include polystyrene, styrene-acrylic copolymers, such as styrene-hexylmethacrylate copolymers, styrene-vinyl toluene copolymers, polyesters, such as PE-200, available from Goodyear, polyurethanes, polyvinylcarbazoles, epoxy resins, phenoxy resins, polyamide resins, polycarbonates, poly-terpenes, silicone elastomers, polyvinylalcohols, such as Gelvatol 20-90, 9000, 20-60, 6000, 20-30, 3000, 40-20, 40-10, 26-90, and 30-30, available from Monsanto Plastics and Resins Co., St. Louis, Mo., polyvinylformals, such as Formvar 12/85, 5/95E, 6/95E, 7/95E, and 15/95E, available from Monsanto Plastics and Resins Co., St. Louis, Mo., polyvinylbutyrals, such as Butvar B-72, B-74, B-73, B-76, B-79, B-90, and B-98, available from Monsanto Plastics and Resins Co., St. Louis, Mo., and the like as well as mixtures

thereof. The softenable layer typically comprises the softenable material in an amount of from about 5 to about 95 percent by weight and the pigment in an amount of from about 5 to about 95 percent by weight, although the relative amounts can be outside this range. Preferably, the softenable layer comprises the softenable material in an amount of from about 40 to about 90 percent by weight and the pigment in an amount of from about 10 to about 60 percent by weight, and more preferably comprises the softenable material in an amount of from about 80 to about 90 percent by weight and the pigment in an amount of from about 10 to 20 percent by weight, although the relative amounts can be outside these ranges.

The migration imaging members may optionally contain a charge transport material in the softenable layers and may also contain a charge transport material in an optional separate charge transport layer. One of the advantages of the present invention, however, is that a charge transport material is not required in either the softenable layer or in any other layer of the imaging member. If present, the charge transport material can be any suitable charge transport material. The charge transport material can be either a hole transport material (transports positive charges) or an electron transport material (transports negative charges). The sign of the charge used to sensitize the migration imaging member during preparation of the master can be of either polarity. Charge transporting materials are well known in the art. Typical charge transporting materials include the following:

Diamine transport molecules of the type described in U.S. Pat. No. 4,306,008, U.S. Pat. 4,304,829, U.S. Pat. 4,233,384, U.S. Pat. No. 4,115,116, U.S. Pat. No. 4,299,897, and U.S. Pat. No. 4,081,274, the disclosures of each of which are totally incorporated herein by reference. Typical diamine transport molecules include N,N'-diphenyl-N,N'-bis(3"-methylphenyl)-(1,1'-biphenyl)-4,4'-diamine, N,N'-diphenyl-N,N'-bis(4-methylphenyl)-(1,1'-biphenyl)-4,4'-diamine, N,N'-diphenyl-N,N'-bis(2-methylphenyl)-(1,1'-biphenyl)-4,4'-diamine, N,N'-diphenyl-N,N'-bis(3-ethylphenyl)-(1,1'-biphenyl)-4,4'-diamine, N,N'-diphenyl-N,N'-bis(4-ethylphenyl)-(1,1'-biphenyl)-4,4'-diamine, N,N'-diphenyl-N,N'-bis(4-n-butylphenyl)-(1,1'-biphenyl)-4,4'-diamine, N,N'-diphenyl-N,N'-bis(3-chlorophenyl)-(1,1'-biphenyl)-4,4'-diamine, N,N'-diphenyl-N,N'-bis(4-chlorophenyl)-(1,1'-biphenyl)-4,4'-diamine, N,N'-diphenyl-N,N'-bis(phenylmethyl)-(1,1'-biphenyl)-4,4'-diamine, N,N'-diphenyl-N,N'-tetraphenyl-[2,2'-dimethyl-1,1'-biphenyl]-4,4'-diamine, N,N',N'-tetra(4-methylphenyl)-[2,2'-dimethyl-1,1'-biphenyl]-4,4'-diamine, N,N'-diphenyl-N,N'-bis(4-methylphenyl)-[2,2'-dimethyl-1,1'-biphenyl]-4,4'-diamine, N,N'-diphenyl-N,N'-bis(2-methylphenyl)-[2,2'-dimethyl-1,1'-biphenyl]-4,4'-diamine, N,N'-diphenyl-N,N'-bis(3-methylphenyl)-[2,2'-dimethyl-1,1'-biphenyl]-4,4'-diamine, N,N'-diphenyl-N,N'-bis(3-methylphenyl)-pyrenyl-1,6-diamine, and the like.

Pyrazoline transport molecules as disclosed in U.S. Pat. No. 4,315,982, U.S. Pat. No. 4,278,746, and U.S. Pat. No. 3,837,851, the disclosures of each of which are totally incorporated herein by reference. Typical pyrazoline transport molecules include 1-[lepidyl-(2)]-3-(p-diethylaminophenyl)-5-(p-diethylaminophenyl)pyrazoline, 1-[quinolyl-(2)]-3-(p-diethylaminophenyl)-5-(p-diethylaminophenyl)pyrazoline, 1-[pyridyl(2)]-3-(p-diethylaminostyryl)-5-(p-diethylaminophenyl)pyrazoline, 1-[6-methoxypyridyl-(2)]-3-(p-diethylaminostyryl)-5-(p-diethylaminophenyl)pyrazoline, 1-phenyl-3-[p-dimethylaminostyryl]-5-(p-dimethylaminostyryl)pyrazoline, 1-phenyl-3-[p-dimethylaminostyryl]pyrazoline,

diethylaminostyryl]-5-(p-diethylaminostyryl)pyrazoline, and the like.

Substituted fluorene charge transport molecules as described in U.S. Pat. No. 4,245,021, the disclosure of which is totally incorporated herein by reference. Typical fluorene charge transport molecules include 9-(4'-dimethylaminobenzylidene)fluorene, 9-(4'-methoxybenzylidene)fluorene, 9-(2',4'-dimethoxybenzylidene)fluorene, 2-nitro-9-benzylidene-fluorene, 2-nitro-9-(4'-diethylaminobenzylidene)fluorene, and the like.

Oxadiazole transport molecules such as 2,5-bis(4-diethylaminophenyl)-1,3,4-oxadiazole, pyrazoline, imidazole, triazole, and the like. Other typical oxadiazole transport molecules are described, for example, in German Patent 1,058,836, German Patent 1,060,260 and German Patent 1,120,875, the disclosures of each of which are totally incorporated herein by reference.

Hydrazone transport molecules, such as p-diethylamino benzaldehyde-(diphenylhydrazone), o-ethoxy-p-diethylaminobenzaldehyde-(diphenylhydrazone), o-methyl-p-diethylaminobenzaldehyde-(diphenylhydrazone), o-methyl-p-dimethylaminobenzaldehyde-(diphenylhydrazone), 1-naphthalenecarbaldehyde 1-methyl-1-phenylhydrazone, 1-naphthalenecarbaldehyde 1,1-phenylhydrazone, 4-methoxynaphthlene-1-carbaldehyde 1-methyl-1-phenylhydrazone, and the like. Other typical hydrazone transport molecules are described, for example in U.S. Pat. No. 4,150,987, U.S. Pat. No. 4,385,106, U.S. Pat. No. 4,338,388, and U.S. Pat. No. 4,387,147, the disclosures of each of which are totally incorporated herein by reference.

Carbazole phenyl hydrazone transport molecules such as 9-methylcarbazole-3-carbaldehyde-1,1-diphenylhydrazone, 9-ethylcarbazole-3-carbaldehyde-1-methyl-1-phenylhydrazone, 9-ethylcarbazole-3-carbaldehyde-1-ethyl-1-phenylhydrazone, 9-ethylcarbazole-3-carbaldehyde-1-ethyl-1-benzyl-1-phenylhydrazone, 9-ethylcarbazole-3-carbaldehyde-1,1-diphenylhydrazone, and the like. Other typical carbazole phenyl hydrazone transport molecules are described, for example, in U.S. Pat. No. 4,256,821 and U.S. Pat. No. 4,297,426, the disclosures of each of which are totally incorporated herein by reference.

Vinyl-aromatic polymers such as polyvinyl anthracene, polyacenaphthylene; formaldehyde condensation products with various aromatics such as condensates of formaldehyde and 3-bromopyrene; 2,4,7-trinitrofluorenone, and 3,6-dinitro-N-t-butylnaphthalimide as described, for example, in U.S. Pat. No. 3,972,717, the disclosure of which is totally incorporated herein by reference.

Oxadiazole derivatives such as 2,5-bis-(p-diethylaminophenyl)-oxadiazole-1,3,4 described in U.S. Pat. No. 3,895,944, the disclosure of which is totally incorporated herein by reference.

Tri-substituted methanes such as alkyl-bis(N,N-dialkylaminoaryl)methane, cycloalkyl-bis(N,N-dialkylaminoaryl)methane, and cycloalkenyl-bis(N,N-dialkylaminoaryl)methane as described in U.S. Pat. No. 3,820,989, the disclosure of which is totally incorporated herein by reference.

5

10

9-Fluorenylidene methane derivatives having the formula



wherein X and Y are cyano groups or alkoxy carbonyl groups; A, B, and W are electron withdrawing groups independently selected from the group consisting of acyl, alkoxy carbonyl, nitro, alkylaminocarbonyl, and derivatives thereof; m is a number of from 0 to 2; and n is the number 0 or 1 as described in U.S. Pat. No. 4,474,865, the disclosure of which is totally incorporated herein by reference. Typical 9-fluorenylidene methane derivatives encompassed by the above formula include (4-n-butoxycarbonyl-9-fluorenylidene)malononitrile, (4-phenethoxycarbonyl-9-fluorenylidene)malononitrile, (4-carboxy-9-fluorenylidene)malononitrile, (4-n-butoxycarbonyl-2,7-dinitro-9-fluorenylidene)malonate, and the like.

Other charge transport materials include poly-1-vinylpyrene, poly-9-vinylanthracene, poly-9-(4-pentenyl)-carbazole, poly-9-(5-hexyl)carbazole, polymethylene pyrene, poly-1-(pyrenyl)-butadiene, polymers such as alkyl, nitro, amino, halogen, and hydroxy substituted polymers such as poly-3-amino carbazole, 1,3-dibromo-poly-N-vinyl carbazole, 3,6-dibromo-poly-N-vinyl carbazole, and numerous other transparent organic polymeric or non-polymeric transport materials as described in U.S. Pat. No. 3,870,516, the disclosure of which is totally incorporated herein by reference. Also suitable as charge transport materials are phthalic anhydride, tetrachlorophthalic anhydride, benzil, mellitic anhydride, S-tricyanobenzene, picryl chloride, 2,4-dinitrochlorobenzene, 2,4-dinitrobromobenzene, 4-nitrobiphenyl, 4,4-dinitrophenyl, 2,4,6-trinitroanisole, trichlorotrinitrobenzene, trinitro-O-toluene, 4,6-dichloro-1,3-dinitrobenzene, 4,6-dibromo-1,3-dinitrobenzene, P-dinitrobenzene, chloranil, bromanil, and mixtures thereof, 2,4,7-trinitro-9-fluorenone, 2,4,5,7-tetrinitrofluorenone, trinitroanthracene, dinitroacridene, tetracyanopyrene, dinitroanthraquinone, polymers having aromatic or heterocyclic groups with more than one strongly electron withdrawing substituent such as nitro, sulfonate, carboxyl, cyano, or the like, including polyesters, polysiloxanes, polyamides, polyurethanes, and epoxies, as well as block, graft, or random copolymers containing the aromatic moiety, and the like, as well as mixtures thereof, as described in U.S. Pat. No. 4,081,274, the disclosure of which is totally incorporated herein by reference.

Also suitable are charge transport materials such as triaryl amines, including trityl amine, of the formula

55

60



and the like, as disclosed in, for example, U.S. Pat. No. 3,240,597 and U.S. Pat. No. 3,180,730, the disclosures of

which are totally incorporated herein by reference, and substituted diarylmethane and triarylmethane compounds, including bis-(4-diethylamino-2-methylphenyl)phenylmethane, of the formula



and the like, as disclosed in, for example, U.S. Pat. No. 4,082,551, U.S. Pat. No. 3,755,310, U.S. Pat. No. 3,647,431, British Patent 984,965, British Patent 980,879, and British Patent 1,141,666, the disclosures of which are totally incorporated herein by reference.

When the charge transport molecules are combined with an insulating binder to form the softenable layer, the amount of charge transport molecule which is used can vary depending upon the particular charge transport material and its compatibility (e.g. solubility) in the continuous insulating film forming binder phase of the softenable matrix layer and the like. Satisfactory results have been obtained using between about 5 percent to about 50 percent by weight charge transport molecule based on the total weight of the softenable layer. A particularly preferred charge transport molecule is one having the general formula



wherein X, Y and Z are selected from the group consisting of hydrogen, an alkyl group having from 1 to about 20 carbon atoms and chlorine, and at least one of X, Y and Z is independently selected to be an alkyl group having from 1 to about 20 carbon atoms or chlorine. If Y and Z are hydrogen, the compound can be named N,N'-diphenyl-N,N'-bis(alkylphenyl)-[1,1'-biphenyl]-4,4'-diamine wherein the alkyl is, for example, methyl, ethyl, propyl, n-butyl, or the like, or the compound can be N,N'-diphenyl-N,N'-bis(chlorophenyl)-[1,1'-biphenyl]-4,4'-diamine. Excellent results can be obtained when the softenable layer containing a charge transport material contains from about 8 percent to about 40 percent by weight of these diamine compounds based on the total weight of the softenable layer. Optimum results are achieved when the softenable layer containing a charge transport material contains from about 16 percent to about 32 percent by weight of N,N'-diphenyl-N,N'-bis(3"-methylphenyl)-(1,1'-biphenyl)-4,4'-diamine based on the total weight of the softenable layer.

The optional charge transport material can be present in the softenable material in any effective amount, generally from about 5 to about 50 percent by weight and preferably from about 8 to about 40 percent by weight. The charge transport material can be incorporated into the softenable layer by any suitable technique. For example, it can be

mixed with the softenable layer components by dissolution in a common solvent. If desired, a mixture of solvents for the charge transport material and the softenable layer material can be employed to facilitate mixing and coating.

- 5 The optional charge transport layer can comprise any suitable film forming binder material. Typical film forming binder materials include styrene acrylate copolymers, polycarbonates, co-polycarbonates, polyesters, co-polyesters, polyurethanes, polyvinyl acetate, polyvinyl butyral, polystyrenes, alkyd substituted polystyrenes, styrene-olefin copolymers, styrene-co-n-hexylmethacrylate, an 80/20 mole percent copolymer of styrene and hexylmethacrylate having an intrinsic viscosity of 0.179 dl/gm; other copolymers of styrene and hexylmethacrylate, styrene-vinyltoluene copolymers, polyalpha-methylstyrene, mixtures thereof, and copolymers thereof. The above group of materials is not intended to be limiting, but merely illustrative of materials suitable as film forming binder materials in the optional charge transport layer. The film forming binder material typically is substantially electrically insulating and does not adversely chemically react during the xeroprinting master making and xeroprinting steps of the present invention. Although the optional charge transport layer has been described as coated on a substrate, in some embodiments, the charge transport layer itself can have sufficient strength and integrity to be substantially self supporting and can, if desired, be brought into contact with a suitable conductive substrate during the imaging process. As is well known in the art, a uniform deposit of electrostatic charge of suitable polarity can be substituted for a substrate. Alternatively, a uniform deposit of electrostatic charge of suitable polarity on the exposed surface of the charge transport spacing layer can be substituted for a conductive substrate layer to facilitate the application of electrical migration forces to the migration layer. This technique of "double charging" is well known in the art. The charge transport layer is of any effective thickness, typically from about 1 to about 25 microns, and preferably from about 2 to about 20 microns, although the thickness can be outside of this range.
- 10 Charge transport molecules suitable for the charge transport layer are described in detail herein. The specific charge transport molecule utilized in the charge transport layer of any given imaging member can be identical to or different from any optional charge transport molecule employed in the softenable layer. Similarly, the concentration of the charge transport molecule utilized in the charge transport spacing layer of any given imaging member can be identical to or different from the concentration of any optional charge transport molecule employed in the softenable layer. When the charge transport material and film forming binder are combined to form the charge transport spacing layer, the amount of charge transport material used can vary depending upon the particular charge transport material and its compatibility (e.g. solubility) in the continuous insulating film forming binder. Satisfactory results have been obtained using between about 5 percent and about 50 percent based on the total weight of the optional charge transport spacing layer, although the amount can be outside of this range. The charge transport material can be incorporated into the charge transport layer by similar techniques to those employed for the softenable layer.
- 15
- 20
- 25
- 30
- 35
- 40
- 45
- 50
- 55
- 60

The optional adhesive layer can include any suitable adhesive material. Typical adhesive materials include copolymers of styrene and an acrylate, polyester resin such as DuPont 49000 (available from E. I. du Pont & de Nemours Company), copolymer of acrylonitrile and vinylidene chloride, polyvinyl acetate, polyvinyl butyral and

the like and mixtures thereof. The adhesive layer can have any effective thickness, typically from about 0.05 micron to about 1 micron, although the thickness can be outside of this range. When an adhesive layer is employed, it preferably forms a uniform and continuous layer having a thickness of about 0.5 micron or less to ensure satisfactory discharge during the xeroprinting process. It can also optionally include charge transport molecules.

The optional charge blocking layer can be of various suitable materials, provided that the objectives of the present invention are achieved, including aluminum oxide, polyvinyl butyral, silane and the like, as well as mixtures thereof. This layer, which is generally applied by known coating techniques, is of any effective thickness, typically from about 0.05 to about 0.5 micron, and preferably from about 0.05 to about 0.1 micron, although the thickness can be outside of this range. Typical coating processes include draw bar coating, spray coating, extrusion, dip coating, gravure roll coating, wire-wound rod coating, air knife coating and the like. This layer can also be applied by lamination techniques as described herein.

The optional overcoating layer can be substantially electrically insulating, or have any other suitable properties. The overcoating preferably is substantially transparent, at least in the spectral region where electromagnetic radiation is used for imagewise exposure step in the master making process and for the uniform exposure step in the xeroprinting process. The overcoating layer is continuous and preferably of a thickness of up to about 1 to 2 microns. More preferably, the overcoating has a thickness of from about 0.1 micron to about 0.5 micron to minimize residual charge buildup. Overcoating layers greater than about 1 to 2 microns thick can also be used. Typical overcoating materials include acrylic-styrene copolymers, methacrylate polymers, methacrylate copolymers, styrene-butylmethacrylate copolymers, butylmethacrylate resins, vinylchloride copolymers, fluorinated homo or copolymers, high molecular weight polyvinyl acetate, organosilicon polymers and copolymers, polyesters, polycarbonates, polyamides, polyvinyl toluene and the like. The overcoating layer generally protects the softenable layer to provide greater resistance to the adverse effects of abrasion during handling, master making, and xeroprinting. The overcoating layer preferably adheres strongly to the softenable layer to minimize damage. The overcoating layer can also have adhesive properties at its outer surface which provide improved resistance to toner filming during toning, transfer, and/or cleaning. The adhesive properties can be inherent in the overcoating layer or can be imparted to the overcoating layer by incorporation of another layer or component of adhesive material. These adhesive materials should not degrade the film forming components of the overcoating and preferably have a surface energy of less than about 20 ergs/cm<sup>2</sup>. Typical adhesive materials include fatty acids, salts and esters, fluorocarbons, silicones, and the like. The coatings can be applied by any suitable technique such as draw bar, spray, dip, melt, extrusion, and gravure coating, vacuum coating, or the like. It will be appreciated that these overcoating layers protect the imaging member before imaging, during imaging, after the members have been imaged, and during xeroprinting if it is used as a xeroprinting master.

The antistatic layer generally comprises a binder and an antistatic agent. The binder and antistatic agent are present in any effective relative amounts, typically from about 5 to about 50 percent by weight antistatic agent and from about 50 to about 95 percent by weight binder, and preferably about 10 percent by weight antistatic agent and about 90

percent by weight binder, although the relative amounts can be outside this range. Typical thicknesses for the antistatic layer are from about 0.5 to about 25 microns, and preferably from about 1 to about 3 microns, although the thickness can be outside these ranges. The antistatic layer can be applied to the imaging member by any desired method, such as draw bar coating, spray coating, extrusion, dip coating, gravure roll coating, wire-wound rod coating, air knife coating, and the like. In one preferred method, the antistatic layer is coated onto the imaging member by a slot extrusion process, wherein a flat die is situated with the die lips in close proximity to the web of the substrate to be coated, resulting in a continuous film of the coating solution evenly distributed across one surface of the sheet, followed by drying in an air dryer at 100° C.

Any suitable or desired binder can be employed. Examples of suitable binders include (a) hydrophilic polysaccharides and their modifications, such as (1) starch (such as starch SLS-280, available from St. Lawrence starch), (2) cationic starch (such as Cato-72, available from National Starch), (3) hydroxyalkylstarch, wherein alkyl has at least one carbon atom and wherein the number of carbon atoms is such that the material is water soluble, preferably from about 1 to about 20 carbon atoms, and more preferably from about 1 to about 10 carbon atoms, such as methyl, ethyl, propyl, butyl, or the like (such as hydroxypropyl starch (#02382, available from Poly Sciences Inc.) and hydroxyethyl starch (#06733, available from Poly Sciences Inc.)), (4) gelatin (such as Calfskin gelatin #00639, available from Poly Sciences Inc.), (5) alkyl celluloses and aryl celluloses, wherein alkyl has at least one carbon atom and wherein the number of carbon atoms is such that the material is water soluble, preferably from 1 to about 20 carbon atoms, more preferably from 1 to about 10 carbon atoms, and even more preferably from 1 to about 7 carbon atoms, such as methyl, ethyl, propyl, butyl, pentyl, hexyl, benzyl, and the like (such as methyl cellulose (Methocel AM 4, available from Dow Chemical Company)), and wherein aryl has at least 6 carbon atoms and wherein the number of carbon atoms is such that the material is water soluble, preferably from 6 to about 20 carbon atoms, more preferably from 6 to about 10 carbon atoms, and even more preferably about 6 carbon atoms, such as phenyl, (6) hydroxy alkyl celluloses, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, benzyl, or the like (such as hydroxyethyl cellulose (Natrinosol 250 LR, available from Hercules Chemical Company), and hydroxypropyl cellulose (Klucel Type E, available from Hercules Chemical Company)), (7) alkyl hydroxy alkyl celluloses, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, benzyl, or the like (such as ethyl hydroxyethyl cellulose (Bermocoll, available from Berol Kem. A. B. Sweden)), (8) hydroxy alkyl alkyl celluloses, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as hydroxyethyl methyl cellulose (HEM, available from British Celanese Ltd., also available as Tylose MH, MHK from Kalle A. G.), hydroxypropyl methyl cellulose (Methocel K35LV, avail-

able from Dow Chemical Company), and hydroxy butylmethyl cellulose (such as HBMC, available from Dow Chemical Company)), (9) dihydroxyalkyl cellulose, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as dihydroxypropyl cellulose, which can be prepared by the reaction of 3-chloro-1, 2-propane with alkali cellulose), (10) hydroxy alkyl hydroxy alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as hydroxypropyl hydroxyethyl cellulose, available from Aqualon Company), (11) halodeoxycellulose, wherein halo represents a halogen atom (such as chlorodeoxycellulose, which can be prepared by the reaction of cellulose with sulfuryl chloride in pyridine at 25° C.), (12) amino deoxy cellulose (which can be prepared by the reaction of chlorodeoxy cellulose with 19 percent alcoholic solution of ammonia for 6 hours at 160° C.), (13) dialkylammonium halide hydroxy alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein halide represents a halogen atom (such as diethylammonium chloride hydroxy ethyl cellulose, available as Celquat H-100, L-200, National Starch and Chemical Company), (14) hydroxyalkyl trialkyl ammonium halide hydroxyalkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein halide represents a halogen atom (such as hydroxypropyl trimethyl ammonium chloride hydroxyethyl cellulose, available from Union Carbide Company as Polymer JR), (15) dialkyl amino alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, (such as diethyl amino ethyl cellulose, available from Poly Sciences Inc. as DEAE cellulose #05178), (16) carboxyalkyl dextrans, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, and the like, (such as carboxymethyl dextrans, available from Poly Sciences Inc. as #16058), (17) dialkyl aminoalkyl dextran, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as diethyl aminoethyl dextran, available from Poly Sciences Inc. as #5178), (18) amino dextran (available from Molecular Probes Inc), (19) carboxy alkyl cellulose salts, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the

like, and wherein the cation is any conventional cation, such as sodium, lithium, potassium, calcium, magnesium, or the like (such as sodium carboxymethyl cellulose CMC 7HOF, available from Hercules Chemical Company), (20) gum arabic (such as #G9752, available from Sigma Chemical Company), (21) carrageenan (such as #C1013 available from Sigma Chemical Company), (22) Karaya gum (such as #G0503, available from Sigma Chemical Company), (23) xanthan (such as Keltrol-T, available from Kelco division of Merck and Company), (24) chitosan (such as #C3646, available from Sigma Chemical Company), (25) carboxyalkyl hydroxyalkyl guar, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as carboxymethyl hydroxypropyl guar, available from Auqualon Company), (26) cationic guar (such as Celanese Jaguars C-14-S, C-15, C-17, available from Celanese Chemical Company), (27) n-carboxyalkyl chitin, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, such as n-carboxymethyl chitin, (28) dialkyl ammonium hydrolyzed collagen protein, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as dimethyl ammonium hydrolyzed collagen protein, available from Croda as Croquats), (29) agar-agar (such as that available from Pfaltz and Bauer Inc), (30) cellulose sulfate salts, wherein the cation is any conventional cation, such as sodium, lithium, potassium, calcium, magnesium, or the like (such as sodium cellulose sulfate #023 available from Scientific Polymer Products), and (31) carboxyalkylhydroxyalkyl cellulose salts, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein the cation is any conventional cation, such as sodium, lithium, potassium, calcium, magnesium, or the like (such as sodium carboxymethylhydroxyethyl cellulose CMHEC 43H and 37L available from Hercules Chemical Company); (b) vinyl polymers, such as (1) poly(vinyl alcohol) (such as Elvanol available from Dupont Chemical Company), (2) poly (vinyl phosphate) (such as #4391 available from Poly Sciences Inc.), (3) poly (vinyl pyrrolidone) (such as that available from GAF Corporation), (4) vinyl pyrrolidone-vinyl acetate copolymers (such as #02587, available from Poly Sciences Inc.), (5) vinyl pyrrolidone-styrene copolymers (such as #371, available from Scientific Polymer Products), (6) poly (vinylamine) (such as #1562, available from Poly Sciences Inc.), (7) poly (vinyl alcohol) alkoxyLATED, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as poly (vinyl alcohol) ethoxylated #6573, available from Poly Sciences Inc.), and (8) poly (vinyl pyrrolidone-dialkylaminoalkyl alkylacrylate), wherein each alkyl has at least one carbon atom and wherein the number of carbon atoms is such that the material is water soluble, preferably from 1 to about 20 carbon atoms, more preferably

from 1 to about 10 carbon atoms, such as methyl, ethyl, propyl, butyl, and the like (such as poly (vinyl pyrrolidone-diethylaminomethylmethacrylate) #16294 and #16295, available from Poly Sciences Inc.); (c) formaldehyde resins, such as (1) melamine-formaldehyde resin (such as BC 309, available from British Industrial Plastics Limited), (2) urea-formaldehyde resin (such as BC777, available from British Industrial Plastics Limited), and (3) alkylated urea-formaldehyde resins, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as methylated urea-formaldehyde resins, available from American Cyanamid Company as Beetle 65); (d) ionic polymers, such as (1) poly (2-acrylamide-2-methyl propane sulfonic acid) (such as #175 available from Scientific Polymer Products), (2) poly (N,N-dimethyl-3,5-dimethylene piperidinium chloride) (such as #401, available from Scientific Polymer Products), and (3) poly (methylene-guanidine) hydrochloride (such as #654, available from Scientific Polymer Products); (e) latex polymers, such as (1) cationic, anionic, and nonionic styrene-butadiene latexes (such as that available from Gen Corp Polymer Products, such as RES 4040 and RES 4100, available from Unocal Chemicals, and such as DL 6672A, DL6638A, and DL6663A, available from Dow Chemical Company), (2) ethylene-vinylacetate latex (such as Airflex 400, available from Air Products and Chemicals Inc.), (3) vinyl acetate-acrylic copolymer latexes (such as synthemul 97-726, available from Reichhold Chemical Inc, Resyn 25-1110 and Resyn 25-1140, available from National Starch Company, and RES 3103 available from Unocal Chemicals; (4) quaternary acrylic copolymer latexes, particularly those of the formula



wherein n is a number of from about 10 to about 100, and preferably about 50, R is hydrogen or methyl, R<sub>1</sub> is hydrogen, an alkyl group, or an aryl group, and R<sub>2</sub> is N<sup>+</sup>(CH<sub>3</sub>)<sub>3</sub>X<sup>-</sup>, wherein X is an anion, such as Cl, Br, I, HSO<sub>3</sub>, SO<sub>3</sub>, CH<sub>2</sub>SO<sub>3</sub>, H<sub>2</sub>PO<sub>4</sub>, HPO<sub>4</sub>, PO<sub>4</sub>, or the like, and the degree of quaternization is from about 1 to about 100 percent, including polymers such as polymethyl acrylate trimethyl ammonium chloride latex, such as HX42-1, available from Interpolymer Corp., or the like; (f) maleic anhydride and maleic acid containing polymers, such as (1) styrene-maleic anhydride copolymers (such as that available as Scriptet from Monsanto, and the SMA series available from Arco), (2) vinyl alkyl ether-maleic anhydride copolymers, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as vinyl methyl ether-maleic anhydride copolymer #173, available from Scientific Polymer Products), (3) alkylene-maleic anhydride copolymers, wherein alkylene has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as ethylene-maleic anhydride copolymer #2308, available from Poly Sciences Inc., also available as EMA from Monsanto Chemical Company), (4) butadiene-maleic acid copolymers (such as #07787, available from Poly Sciences Inc.), (5) vinylalky-

lether-maleic acid copolymers, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as vinylmethylether-maleic acid copolymer, available from GAF Corporationas Gantrez S-95), and (6) alkyl vinyl ether-maleic acid esters, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as methyl vinyl ether-maleic acid ester #773, available from Scientific Polymer Products); (g) acrylamide containing polymers, such as (1) poly (acrylamide) (such as #02806, available from Poly Sciences Inc.), (2) acrylamide-acrylic acid copolymers (such as #04652, #02220, and #18545, available from Poly Sciences Inc.), and (3) poly (N,N-dimethyl acrylamide) (such as #004590, available from Poly Sciences Inc.); and (h) poly (alkylene imine) containing polymers, wherein alkylene has two (ethylene), three (propylene), or four (butylene) carbon atoms, such as (1) poly(ethylene imine) (such as #135, available from Scientific Polymer Products), (2) poly(ethylene imine) epichlorohydrin (such as #634, available from Scientific Polymer Products), and (3) alkoxylated poly (ethylene imine), wherein alkyl has one (methoxylated), two (ethoxylated), three (propoxylated), or four (butoxylated) carbon atoms (such as ethoxylated poly (ethylene imine) #636, available from Scientific Polymer Products); and the like. Any mixtures of the above ingredients in any relative amounts can also be employed.

Any desired or suitable antistatic agent can be employed. Examples of suitable antistatic agents include amine acid salts and quaternary choline halides. Examples of suitable aliphatic amine acid salts include acid salts of aliphatic primary amines, such as (I) acid salts of aliphatic diamines, of the general formula H<sub>2</sub>N(R<sub>1</sub>)NH<sub>2</sub>.H<sub>n</sub>X<sup>n-</sup>, wherein R<sub>1</sub> can be (but is not limited to) alkyl, substituted alkyl (such as imino alkyl imine, imino alkyl imino carbonyl, dialkyl imine, or the like), alkylene, substituted alkylene (such as alkylene imine, oxyalkylene, alkylene carbonyl, mercapto alkylene, or the like), imine, diamino imine, and carbonyl, X is an anion, such as Cl<sup>-</sup>, Br<sup>-</sup>, I<sup>-</sup>, HSO<sub>4</sub><sup>2-</sup>, SO<sub>4</sub><sup>2-</sup>, NO<sub>3</sub><sup>-</sup>, HCOO<sup>-</sup>, CH<sub>3</sub>COO<sup>-</sup>, HCO<sub>3</sub><sup>-</sup>, CO<sub>3</sub><sup>2-</sup>, H<sub>2</sub>PO<sub>4</sub><sup>-</sup>, HPO<sub>4</sub><sup>2-</sup>, PO<sub>4</sub><sup>3-</sup>, SCN<sup>-</sup>, BF<sub>4</sub><sup>-</sup>, ClO<sub>4</sub><sup>-</sup>, SSO<sub>3</sub><sup>-</sup>, CH<sub>3</sub>SO<sub>3</sub><sup>-</sup>, CH<sub>3</sub>C<sub>6</sub>H<sub>4</sub>SO<sub>3</sub><sup>-</sup>, or the like, as well as mixtures thereof, and n is an integer of 1, 2, or 3, including (a) guanidine compounds, such as (1) guanidine hydrochloride [H<sub>2</sub>NC(=NH)NH<sub>2</sub>.HCl] (Aldrich 17,725-3, G1,170-5); (2) guanidine sulfate [H<sub>2</sub>NC(=NH)NH<sub>2</sub>]<sub>2</sub>.H<sub>2</sub>SO<sub>4</sub> (Aldrich 30,739-4); (3) guanidine nitrate [H<sub>2</sub>NC(=NH)NH<sub>2</sub>.HNO<sub>3</sub>] (Aldrich 23,424-9); (4) guanidine carbonate [H<sub>2</sub>NC(=NH)NH<sub>2</sub>]<sub>2</sub>.H<sub>2</sub>CO<sub>3</sub> (Aldrich G1,165-9); (5) guanidine thiocyanate [H<sub>2</sub>NC(=NH)NH<sub>2</sub>.HSCN] (Aldrich 29,288-5); (6) amino guanidine bicarbonate [H<sub>2</sub>NNHC(=NH)NH<sub>2</sub>.H<sub>2</sub>CO<sub>3</sub>] (Aldrich 10,926-6); (7) amino guanidine nitrate [H<sub>2</sub>NNHC(=NH)NH<sub>2</sub>.HNO<sub>3</sub>] (Aldrich A5,610-8); (8) amino guanidine hemisulfate [NH<sub>2</sub>NHC(=NH)NH<sub>2</sub>]<sub>2</sub>.H<sub>2</sub>SO<sub>4</sub> (Kodak 4023, available from Eastman Kodak Co.); (9) 1,3-diamino guanidine monohydrochloride [H<sub>2</sub>NNHC(=NH)NNH<sub>2</sub>.HCl] (Aldrich 14,341-3); (10) N-guanyl urea sulfate hydrate [H<sub>2</sub>NC(=NH)NHCONH<sub>2</sub>]<sub>2</sub>.H<sub>2</sub>SO<sub>4</sub>.xH<sub>2</sub>O (Aldrich 27,345-7); (11) (4-amino butyl) guanidine sulfate H<sub>2</sub>N(CH<sub>2</sub>)<sub>4</sub>NHC(=NH)NH<sub>2</sub>.H<sub>2</sub>SO<sub>4</sub> (Aldrich 10,144-3); (12) malonamamidine hydrochloride

$\text{H}_2\text{NC}(=\text{NH})\text{CH}_2\text{CONH}_2\text{HCl}$  (Aldrich 17,651-6); and the like; (b) alkylene compounds, such as (1) ethylene diamine dihydrochloride  $\text{H}_2\text{N}(\text{CH}_2)_2\text{NH}_2\text{HCl}$  (Aldrich 19,580-4); (2) 1,3-diaminopropane dihydrochloride  $\text{H}_2\text{N}(\text{CH}_2)_3\text{NH}_2\text{HCl}$  (Aldrich D2,380-7); (3) 1,4-diamino butane dihydrochloride  $\text{H}_2\text{N}(\text{CH}_2)_4\text{NH}_2\text{HCl}$  (Aldrich 23,400-1); (4) 1,5-diamino pentane dihydrochloride  $\text{H}_2\text{N}(\text{CH}_2)_5\text{NH}_2\text{HCl}$  (Aldrich 27,182-9); (5) 1,6-diamine hexane dihydrochloride  $\text{H}_2\text{N}(\text{CH}_2)_6\text{NH}_2\text{HCl}$  (Aldrich 24,713-1); (6) triethylene tetramine dihydrochloride  $\text{H}_2\text{N}(\text{CH}_2)_2\text{NH}(\text{CH}_2)_2\text{NH}(\text{CH}_2)_2\text{NH}_2\text{HCl}$  (Aldrich 29,951-0); (7) triethylene tetramine tetrahydrochloride  $\text{H}_2\text{N}(\text{CH}_2)_2\text{NH}(\text{CH}_2)_2\text{NH}(\text{CH}_2)_2\text{NH}_2\text{HCl}$  (Aldrich 16,196-9); (8) spermine tetrahydrochloride  $\text{H}_2\text{N}(\text{CH}_2)_3\text{NH}(\text{CH}_2)_4\text{NH}_2\text{HCl}$  (Aldrich 28,716-4); (9) spermidine trihydrochloride  $\text{H}_2\text{N}(\text{CH}_2)_4\text{NH}(\text{CH}_2)_3\text{NH}_2\text{HCl}$  (Aldrich 23,399-4); (10) cystamine dihydrochloride  $\text{S}_2(\text{CH}_2\text{CH}_2\text{NH}_2)_2\text{HCl}$  (Aldrich C12,150-9); (11) 2,2'-oxybis (ethylamine) dihydrochloride  $\text{O}(\text{CH}_2\text{CH}_2\text{NH}_2)_2\text{HCl}$  (Aldrich 17,609-5); (12) glycamide hydrochloride  $\text{H}_2\text{NCH}_2\text{CONH}_2\text{HCl}$  (Aldrich G610-4); (13) 1,3-diamino acetone dihydrochloride monohydrate  $\text{H}_2\text{NCH}_2\text{COCH}_2\text{NH}_2\text{HCl}\text{H}_2\text{O}$  (Aldrich 23,244-0); (14) urea sulfate  $(\text{H}_2\text{NCONH}_2)_2\text{H}_2\text{SO}_4$  (Aldrich 28,059-3); (15) urea phosphate  $\text{H}_2\text{NCONH}_2\text{H}_3\text{PO}_4$  (Aldrich 29,282-6); (16) 2,2-dimethyl-1,3-propane diamine dihydrochloride  $\text{H}_2\text{NCH}_2\text{C}(\text{CH}_3)_2\text{CH}_2\text{NH}_2\text{HCl}$  (Aldrich 22,693-9); (17) 1,4-diamino-2-butane dihydrochloride  $\text{H}_2\text{NCH}_2\text{CH}_2\text{COCH}_2\text{CH}_2\text{NH}_2\text{HCl}$  (Aldrich 19, 933-8); (18) L-leucinamide hydrochloride  $(\text{CH}_3)_2\text{CHCH}_2\text{CH}(\text{NH}_2)\text{CONH}_2\text{HCl}$  (Aldrich 28,642-7); (19) (2-aminoethyl) trimethyl ammonium chloride hydrochloride  $\text{H}_2\text{NCH}_2\text{CH}_2\text{N}(\text{CH}_3)_3\text{Cl}\text{HCl}$  (Aldrich 28,455-6); and the like; (II) acid salts of aliphatic monoamines, of the general formula  $\text{R}_2\text{NH}_2\text{H}_n\text{X}^{n-}$ , wherein  $\text{R}_2$  can be (but is not limited to) alkyl, substituted alkyl (such as alkyl imine, alkoxy alkyl imine, alkyl amino imine, halogenated alkyl imine, alkyl mercaptylimine, alkylamine alkoxy amine, alkyl mercapto amine, halogenated alkyl amine, halogenated alkyl amide, alkyl ester, allyl alkyl amine, alkyl mercaptylester, and the like), alkylene, substituted alkylene (such as alkylene imine, alkylene ester, and the like), imine, amine, substituted amine (such as hydroxylamine, alkyne hydroxyl amino, halogenated amine, and the like), anhydride ester, and the like,  $\text{X}$  is an anion, such as  $\text{Cl}^-$ ,  $\text{Br}^-$ ,  $\text{I}^-$ ,  $\text{HSO}_4^-$ ,  $\text{SO}_4^{2-}$ ,  $\text{NO}_3^-$ ,  $\text{HCOO}^-$ ,  $\text{CH}_3\text{COO}^-$ ,  $\text{HCO}_3^-$ ,  $\text{CO}_3^{2-}$ ,  $\text{H}_2\text{PO}_4^-$ ,  $\text{HPO}_4^{2-}$ ,  $\text{PO}_4^{3-}$ ,  $\text{SCN}^-$ ,  $\text{BF}_4^-$ ,  $\text{ClO}_4^-$ ,  $\text{SSO}_3^-$ ,  $\text{CH}_3\text{SO}_3^-$ ,  $\text{CH}_3\text{C}_6\text{H}_4\text{SO}_3^-$ , or the like, as well as mixtures thereof, and  $n$  is an integer of 1, 2, or 3, including (a) guanidine compounds, such as (1) formamidine hydrochloride  $\text{HC}(=\text{NH})\text{NH}_2\text{HCl}$  (Aldrich 26,860-7); (2) formamidine disulfide dihydrochloride  $[-\text{SC}(=\text{NH})\text{NH}_2]_2\text{HCl}$  (Aldrich 21,946-0); (3) formamidine acetate  $\text{HC}(=\text{NH})\text{NH}_2\text{CH}_3\text{COOH}$  (Aldrich F1,580-3); (4) acetamidine hydrochloride  $\text{CH}_3\text{C}(=\text{NH})\text{NH}_2\text{HCl}$  (Aldrich 15,915-8); (5) acetamidine acetate  $\text{H}_3\text{CC}(=\text{NH})\text{NH}_2\text{CH}_3\text{COOH}$  (Aldrich 26,997-2); (6) 2-ethyl-2-thiopseudourea hydrobromide  $\text{C}_2\text{H}_5\text{SC}(=\text{NH})\text{NH}_2\text{HBr}$  (Aldrich 30,131-0); (7) guanidine acetic acid  $[\text{H}_2\text{NC}(=\text{NH})\text{NHCH}_2\text{COOH}]$  (Aldrich G1,160-8); (8) 1,1-dimethyl biguanide hydrochloride  $[(\text{CH}_3)_2\text{NC}(=\text{NH})\text{NHC}(=\text{NH})\text{NH}_2\text{HCl}]$  (Aldrich D15, 095-9); (9) 1-methyl guanidine hydrochloride  $\text{CH}_3\text{NHC}(=\text{NH})\text{NH}_2\text{HCl}$  (Aldrich 22,240-2); (10) methyl guanidine sulfate  $[\text{CH}_3\text{NHC}(=\text{NH})\text{NH}_2]_2\text{H}_2\text{SO}_4$  (Kodak 1482, available from Eastman Kodak Co.); (11) 1-ethyl guanidine hydrochloride  $\text{C}_2\text{H}_5\text{NHC}(=\text{NH})\text{NH}_2\text{HCl}$  (Ald-

rich 29,489-6); (12) 1-ethyl guanidine sulfate  $[\text{C}_2\text{H}_5\text{NHC}(=\text{NH})\text{NH}_2]_2\text{H}_2\text{SO}_4$  (Aldrich 27,555-7); (13) dodecyl guanidine hydrochloride  $[\text{CH}_3(\text{CH}_2)_{11}\text{HNC}(=\text{NH})\text{NH}_2\text{HCl}]$  (Betz Paper Company 5 Slimetrol RX=31, 32); (14) 1-(2,2-diethoxyethyl) guanidine sulfate  $[(\text{C}_2\text{H}_5\text{O})_2\text{CHCH}_2\text{NHC}(=\text{NH})\text{NH}_2]_2\text{H}_2\text{SO}_4$  (Aldrich 19,790-4); (15) methyl glyoxal bis (guanyl hydrazone) dihydrochloride hydrate  $\text{CH}_3\text{Cl}=\text{NNHC}(=\text{NH})\text{NH}_2\text{CH}[\text{==NNHC}(=\text{NH})\text{NH}_2]_2\text{HCl}\text{xH}_2\text{O}$  (Aldrich 13,949-1); (16) 2-ethyl-2-thiopseudourea hydrobromide  $\text{C}_2\text{H}_5\text{SC}(=\text{NH})\text{NH}_2\text{HBr}$  (Aldrich 30,131-0); (17) 2-methyl-2-thiopseudourea sulfate  $[\text{CH}_3\text{SC}(=\text{NH})\text{NH}_2]_2\text{H}_2\text{SO}_4$  (Aldrich M8,444-5); (18) o-methyl isourea hydrogen sulfate  $\text{CH}_3\text{OC}(=\text{NH})\text{NH}_2\text{H}_2\text{SO}_4$  (Aldrich M5,370-1); (19) S,S'-15 (1,3-propanediyl) bis (isothiouronium bromide)  $\text{CH}_2[\text{CH}_2\text{SC}(=\text{NH})\text{NH}_2]_2\text{HBr}$  (Aldrich 24,318-3); and the like; (b) alkyl amines, such as (1) methyl amine hydrochloride  $\text{CH}_3\text{NH}_2\text{HCl}$  (Aldrich 12,970-4); (2) ethyl amine hydrochloride  $\text{C}_2\text{H}_5\text{NH}_2\text{HCl}$  (Aldrich 23,283-1); (3) 20 3-chloropropylamine hydrochloride  $\text{Cl}(\text{CH}_2)_3\text{NH}_2\text{HCl}$  (Aldrich 14,254-9); (4) aminomethyl cyclopropane hydrochloride  $\text{C}_3\text{H}_5\text{CH}_2\text{NH}_2\text{HCl}$  (Aldrich A6,380-5); (5) 2-methyl allyl amine hydrochloride  $\text{H}_2\text{C}=\text{C}(\text{CH}_3)\text{CH}_2\text{NH}_2\text{HCl}$  (Aldrich 27,906-4); (6) amino acetonitrile hydrochloride  $\text{H}_2\text{N}(\text{CH}_2\text{CN})\text{HCl}$  (Aldrich 13,052-4); (7) amino acetonitrile bisulfate  $\text{H}_2\text{N}(\text{CH}_2\text{CN})\text{H}_2\text{SO}_4$  (Aldrich 27,999-4); (8) 25 tert-butyl hydrazine hydrochloride  $(\text{CH}_3)_3\text{CNHNH}_2\text{HCl}$  (Aldrich 19,497-2); (9) methoxyl amine hydrochloride  $\text{CH}_3\text{ONH}_2\text{HCl}$  (Aldrich 22,551-7); (10) ethanol amine hydrochloride  $\text{H}_2\text{NCH}_2\text{CH}_2\text{OH}\text{HCl}$  (Aldrich 23,638-1); (11) 0-(tert butyl) hydroxylamine hydrochloride  $(\text{CH}_3)_3\text{CONH}_2\text{HCl}$  (Aldrich 34,006-5); (12) 6-amino-2-methyl-2-heptanol hydrochloride  $\text{CH}_3\text{CH}(\text{NH}_2)(\text{CH}_2)_3\text{C}(\text{CH}_3)_2\text{OH}\text{HCl}$  (Aldrich 29,620-1); (13) o-allyl hydroxyl amine hydrochloride hydrate  $\text{H}_2\text{C}=\text{CHCH}_2\text{ONH}_2\text{HCl}\text{xH}_2\text{O}$  (Aldrich 25,456-8); (14) 30 hydroxylamine hydrochloride  $\text{H}_2\text{NOH}\text{HCl}$  (Aldrich 25,558-0; 15,941-7); (15) hydroxylamine phosphate  $(\text{H}_2\text{NOH})_3\text{H}_3\text{PO}_4$  (Aldrich 34,235-1); (16) hydroxylamine sulfate  $(\text{H}_2\text{NOH})_2\text{H}_2\text{SO}_4$  (Aldrich 21,025-1); (17) D,L-serinol hydrochloride  $\text{H}_2\text{NCH}(\text{CH}_2\text{OH})_2\text{HCl}$  (Aldrich 28,715-6); (18) 2-(ethylthio) ethylamine hydrochloride  $\text{C}_2\text{H}_5\text{SCH}_2\text{CH}_2\text{NH}_2\text{HCl}$  (Aldrich 12,042-1); (19) o-ethyl hydroxylamine hydrochloride  $\text{C}_2\text{H}_5\text{ONH}_2\text{HCl}$  (Aldrich 27,499-2); (20) tris (hydroxymethyl) aminomethane hydrochloride  $(\text{HOCH}_2)_3\text{CNH}_2\text{HCl}$  (Aldrich 85,764-5); (21) octadecylamine hydrochloride  $\text{CH}_2(\text{CH}_2)_{17}\text{NH}_2\text{HCl}$  (Kodak 9209, available from Eastman Kodak Co.); (22) 40 2-aminoethyl hydrogen sulfate  $\text{NH}_2\text{CH}_2\text{CH}_2\text{OSO}_3\text{H}$  (Kodak P5895, available from Eastman Kodak Co.); (23) 2-aminoethane thiosulfuric acid  $\text{NH}_2\text{CH}_2\text{CH}_2\text{SSO}_3\text{H}$  (Kodak 8413, available from Eastman Kodak Co.); (24) 2-bromoethylamine hydrobromide  $\text{BrCH}_2\text{CH}_2\text{NH}_2\text{HBr}$  (Kodak 5020, available from Eastman Kodak Co.); and the like; (c) ester compounds, such as (1) glycine methylester hydrochloride  $\text{H}_2\text{NCH}_2\text{COOCH}_3\text{HCl}$  (Aldrich G-660-0); (2) L-methionine methyl ester hydrochloride  $\text{CH}_3\text{SCH}_2\text{CH}_2\text{CH}(\text{NH}_2)\text{COOCH}_3\text{HCl}$  (Aldrich 86,040-9); (3) L-alanine methyl ester hydrochloride  $\text{CH}_3\text{CH}(\text{NH}_2)\text{COOCH}_3\text{HCl}$  (Aldrich 33,063-9); (4) L-leucine methyl ester hydrochloride  $(\text{CH}_3)_2\text{CHCH}_2\text{CH}(\text{NH}_2)\text{COOCH}_3\text{HCl}$  (Aldrich L100-2); (5) 55 glycine ethyl ester hydrochloride  $\text{H}_2\text{NCH}_2\text{COOC}_2\text{H}_5\text{HCl}$  (Aldrich G650-3); (6)  $\beta$ -alanine ethyl ester hydrochloride  $\text{H}_2\text{N}(\text{CH}_2)_2\text{COOC}_2\text{H}_5\text{HCl}$  (Aldrich 30,614-2); (7) ethyl 4-aminobutyrate hydrochloride  $\text{H}_2\text{N}(\text{CH}_2)_3\text{COOC}_2\text{H}_5\text{HCl}$  (Aldrich E1,060-2); (8) alanine 60

ethyl ester hydrochloride  $\text{CH}_3\text{CH}(\text{NH}_2)\text{COOC}_2\text{H}_5\text{.HCl}$  (Aldrich 26,886-0; 85,566-9); (9) L-methionine ethyl ester hydrochloride  $\text{CH}_3\text{SCH}_2\text{CH}_2\text{CH}(\text{NH}_2)\text{COOC}_2\text{H}_5\text{.HCl}$  (Aldrich 22,067-1); (10) glycine tert butyl ester hydrochloride  $\text{H}_2\text{NCH}_2\text{COOC}(\text{CH}_3)_3\text{.HCl}$  (Aldrich 34,795-7); (11) L-valine ethyl ester hydrochloride  $(\text{CH}_3)_2\text{CHCH}(\text{NH}_2)\text{COOC}_2\text{H}_5\text{.HCl}$  (Aldrich 22,069-8); (12) L-valine methylester hydrochloride  $(\text{CH}_3)_2\text{CHCH}(\text{NH}_2)\text{COOCH}_3\text{.HCl}$  (Aldrich 86,027-1); (13) N- $\alpha$ -acetyl-L-lysine methylester hydrochloride  $\text{H}_2\text{N}(\text{CH}_2)_4\text{CH}(\text{NHCOCH}_3)\text{COOCH}_3\text{.HCl}$  (Aldrich 85,909-5); (14) methyl 5-aminolevulinate hydrochloride  $\text{H}_2\text{NCH}_2\text{COCH}_2\text{COOCH}_3\text{.HCl}$  (Aldrich 28,506-4); and the like.

Also suitable are acid salts of aliphatic secondary amines, such as (III) those of the general formula  $\text{R}_3\text{R}_4\text{NH}.\text{H}_n\text{X}^{n-}$ , wherein  $\text{R}_3$  and  $\text{R}_4$  each, independently of one another, can be (but are not limited to) alkyl (including cyclic alkyl), substituted alkyl (such as hydroxyalkyl, alkoxy alkyl, alkyl nitride, alkylene alkyl, or the like), alkylene, substituted alkylene (such as alkoxy alkylene or the like), hydroxyl, nitrile, oxyalkyl, oxyalkylene, and the like, X is an anion, such as  $\text{Cl}^-$ ,  $\text{Br}^-$ ,  $\text{I}^-$ ,  $\text{HSO}_4^-$ ,  $\text{SO}_4^{2-}$ ,  $\text{NO}_3^-$ ,  $\text{HCOO}^-$ ,  $\text{CH}_3\text{COO}^-$ ,  $\text{HCO}_3^-$ ,  $\text{CO}_3^{2-}$ ,  $\text{H}_2\text{PO}_4^-$ ,  $\text{HPO}_4^{2-}$ ,  $\text{PO}_4^{3-}$ ,  $\text{SCN}^-$ ,  $\text{BF}_4^-$ ,  $\text{ClO}_4^-$ ,  $\text{SSO}_3^-$ ,  $\text{CH}_3\text{SO}_3^-$ ,  $\text{CH}_3\text{C}_6\text{H}_4\text{SO}_3^-$ , or the like, as well as mixtures thereof, and n is an integer of 1, 2, or 3, including (1) dimethylamine hydrochloride  $(\text{CH}_3)_2\text{NH}.\text{HCl}$  (Aldrich 12,636-5); (2) diethyl amine hydrochloride  $(\text{C}_2\text{H}_5)_2\text{NH}.\text{HCl}$  (Aldrich 12,774-4); (3) diethyl amine hydrobromide  $(\text{C}_2\text{H}_5)_2\text{NH}.\text{HBr}$  (Aldrich 31,090-5); (4) diethyl amine phosphate  $(\text{C}_2\text{H}_5)_2\text{NH}.\text{H}_3\text{PO}_4$  (Aldrich 14,115-1); (5) N-propylcyclopropane methyl amine hydrochloride  $\text{C}_3\text{H}_5\text{CH}_2\text{NHCH}_2\text{CH}_2\text{CH}_3\text{.HCl}$  (Aldrich 22,758-7); (6) isopropyl formimidate hydrochloride  $\text{HC}(\text{=NH})\text{OCH}(\text{CH}_3)_2\text{.HCl}$  (Aldrich 34,624-1); (7) N-isopropyl hydroxylamine hydrochloride  $(\text{CH}_3)_2\text{CHNHOH}.\text{HCl}$  (Aldrich 24,865-7); (8) N-(tert butyl) hydroxylamine hydrochloride  $(\text{CH}_3)_3\text{CNHOH}.\text{HCl}$  (Aldrich 19,475-1); (9) dimethyl suberimidate dihydrochloride  $\text{CH}_3\text{OC}(\text{=NH})(\text{CH}_2)_6\text{C}(\text{=NH})\text{OCH}_3\text{.2HCl}$  (Aldrich 17,952-3); (10) N-methylhydroxylamine hydrochloride  $\text{CH}_3\text{NHOH}.\text{HCl}$  (Aldrich M5,040); (11) methyl amino acetonitrile hydrochloride  $\text{CH}_3\text{NHCH}_2\text{CN}.\text{HCl}$  (Aldrich M2,810-3); (12) N-cyclohexyl hydroxylamine hydrochloride  $\text{C}_6\text{H}_{11}\text{NHOH}.\text{HCl}$  (Aldrich 18,646-5); (13) dimethyl adipimidate dihydrochloride  $\text{CH}_3\text{OC}(\text{=NH})(\text{CH}_2)_4\text{C}(\text{=NH})\text{OCH}_3\text{.2HCl}$  (Aldrich 28,562-5); and the like.

Also suitable are acid salts of aliphatic tertiary amines, such as (IV) those of the general formula  $\text{R}_5\text{R}_6\text{R}_7(\text{N})\text{H}_n\text{X}^{n-}$ , wherein  $\text{R}_5$ ,  $\text{R}_6$ , and  $\text{R}_7$  each, independently of one another, can be (but are not limited to) alkyl, substituted alkyl (such as hydroxyalkyl, alkyl halide, alkyl carbonyl, and the like), alkylene, substituted alkylene (such as hydroxy alkylene and the like), alkoxy, thiol, carboxyl, and the like, X is an anion, such as  $\text{Cl}^-$ ,  $\text{Br}^-$ ,  $\text{I}^-$ ,  $\text{HSO}_4^-$ ,  $\text{SO}_4^{2-}$ ,  $\text{NO}_3^-$ ,  $\text{HCOO}^-$ ,  $\text{CH}_3\text{COO}^-$ ,  $\text{HCO}_3^-$ ,  $\text{CO}_3^{2-}$ ,  $\text{H}_2\text{PO}_4^-$ ,  $\text{HPO}_4^{2-}$ ,  $\text{PO}_4^{3-}$ ,  $\text{SCN}^-$ ,  $\text{BF}_4^-$ ,  $\text{ClO}_4^-$ ,  $\text{SSO}_3^-$ ,  $\text{CH}_3\text{SO}_3^-$ ,  $\text{CH}_3\text{C}_6\text{H}_4\text{SO}_3^-$ , or the like, as well as mixtures thereof, and n is an integer of 1, 2, or 3, including (1) trimethylamine hydrochloride  $(\text{CH}_3)_3\text{N}.\text{HCl}$  (Aldrich T7,276-1); (2) triethylamine hydrochloride  $(\text{C}_2\text{H}_5)_3\text{N}.\text{HCl}$  (Aldrich 26,815-1); (3) triethanol amine hydrochloride  $(\text{HOCH}_2\text{CH}_2)_3\text{N}.\text{HCl}$  (Aldrich 15,891-7); (4) 2-dimethyl amino isopropyl chloride hydrochloride  $\text{CH}_3\text{CH}(\text{Cl})\text{CH}_2\text{N}(\text{CH}_3)_2\text{.HCl}$  (Aldrich D14,240-9); (5) 2-dimethyl amino ethyl chloride hydrochloride  $(\text{CH}_3)_2\text{NCH}_2\text{CH}_2\text{Cl}.\text{HCl}$  (Aldrich D14,120-8); (6) 3-dim-

ethyl amino-2-methyl propyl chloride hydrochloride  $(\text{CH}_3)_2\text{NCH}_2\text{CH}(\text{CH}_3)\text{CH}_2\text{Cl}.\text{HCl}$  (Aldrich 15,289-7); (7) 2-dimethyl aminoethanethiol hydrochloride  $(\text{CH}_3)_2\text{NCH}_2\text{CH}_2\text{SH}.\text{HCl}$  (Aldrich D14,100-3); (8) N,N-dimethyl glycine hydrochloride  $(\text{CH}_3)_2\text{NCH}_2\text{COOH}.\text{HCl}$  (Aldrich 21,960-6); (9) 4-(dimethyl amino) butyric acid hydrochloride  $(\text{CH}_3)_2\text{N}(\text{CH}_2)_3\text{COOH}.\text{HCl}$  (Aldrich 26,373-7); (10) N,N-dimethyl hydroxylamine hydrochloride  $\text{HON}(\text{CH}_3)_2\text{.HCl}$  (Aldrich 22,145-7); (11) N,O-dimethyl hydroxylamine hydrochloride  $\text{CH}_3\text{ONHCH}_3\text{.HCl}$  (Aldrich D16,3780-8); (12) 3-[bis(2-hydroxyethyl) amino]-2-hydroxy-1-propane sulfonic acid  $(\text{HOCH}_2\text{CH}_2)_2\text{NCH}_2\text{CH}_2\text{SO}_3\text{H}$  (Aldrich 34,004-9); (13) 2,3-bis (hydroxyamino)-2,3-dimethyl butane sulfate  $(\text{CH}_3)_2\text{C}(\text{NHOH})\text{C}(\text{NHOH})(\text{CH}_3)_2\text{H}_2\text{SO}_4$  (Kodak 11659, available from Eastman Kodak Co.); (14) N,N-bis (2-hydroxyethyl)-2-amino ethane sulfonic acid  $(\text{HOCH}_2\text{CH}_2)_2\text{NCH}_2\text{CH}_2\text{SO}_3\text{H}$  (Kodak 14999, available from Eastman Kodak Co.); and the like.

Also suitable are (V) acid salts of cyclic aliphatic amines, such as

(1)  $(\pm)$ - $\alpha$ -amino- $\gamma$ -butyrolactone hydrobromide (Aldrich A4, 450-9), of the formula



(2) D,L-homocysteine thiolactone hydrochloride (Aldrich H1,580-2), of the formula



(3)  $(\pm)$ -endo-2-aminonorbornane hydrochloride (Aldrich 13,351-5), of the formula



(4) N-ethyl-3-phenyl-2-norbornanamine hydrochloride (Aldrich 17, 951-5), of the formula



(5) 1-adamantanamine hydrochloride (Aldrich 11,519-3), of the formula



(6) 1,3-adamantane diamine dihydrochloride (Aldrich 34, 081-2), of the formula



(7) 3-noradamantanamine hydrochloride (Aldrich 29, 187-0), of the formula



(8) 9-aminofluorene hydrochloride (Aldrich A5,560-8), of the formula



and the like.

Also suitable are acid salts of aromatic amines, such as (VI) acid salts of aromatic amines having both  $-\text{NH}_2$  and  $-\text{OH}$  groups, such as (1)  $(\pm)$ -octopamine hydrochloride  $\text{HOC}_6\text{H}_4\text{CH}(\text{CH}_2\text{NH}_2)\text{OH} \cdot \text{HCl}$  (Aldrich 13,051-6); (2)  $(\pm)$ -norphenylephrine hydrochloride  $\text{HOC}_6\text{H}_4\text{CH}(\text{CH}_2\text{NH}_2)\text{OH} \cdot \text{HCl}$  (Aldrich 11,372-7); (3) norephedrine hydrochloride  $\text{C}_6\text{H}_5\text{CH}(\text{OH})\text{CH}(\text{CH}_3)\text{NH}_2 \cdot \text{HCl}$  (Aldrich 13,143-1, 19,362-3); (4) norepinephrine hydrochloride  $(\text{HO})_2\text{C}_6\text{H}_3\text{CH}(\text{CH}_2\text{NH}_2)\text{OH} \cdot \text{HCl}$  (Aldrich 17,107-7); (5) (1R,2R)- $(-)$ -norpseudoephedrine hydrochloride  $\text{C}_6\text{H}_5\text{CH}(\text{OH})\text{CH}(\text{CH}_3)\text{NH}_2 \cdot \text{HCl}$  (Aldrich 19,363-1); (6)  $(\pm)$ - $\alpha$ -(1-aminoethyl)-4-hydroxybenzyl alcohol hydrochloride  $\text{HOC}_6\text{H}_4\text{CH}[\text{CH}(\text{NH}_2)\text{CH}_3]\text{OH} \cdot \text{HCl}$  (Aldrich A5,445-8); (7) 2-[2-(aminomethyl) phenylthio] benzylalcohol hydrochloride  $\text{H}_2\text{NCH}_2\text{C}_6\text{H}_4\text{SC}_6\text{H}_4\text{CH}_2\text{OH} \cdot \text{HCl}$  (Aldrich 34,632-2); (8) 1-amino-2-naphthol hydrochloride  $\text{H}_2\text{NC}_{10}\text{H}_6\text{OH} \cdot \text{HCl}$  (Aldrich 13,347-7); (9) 4-amino-1-naphthol hydrochloride  $\text{H}_2\text{NC}_{10}\text{H}_6\text{OH} \cdot \text{HCl}$  (Aldrich 13,348-5); (10) tyramine hydrochloride  $\text{HOC}_6\text{H}_4\text{CH}_2\text{CH}_2\text{NH}_2 \cdot \text{HCl}$  (Aldrich T9,035-2); (11) L-tyrosine hydrochloride  $\text{HOC}_6\text{H}_4\text{CH}_2\text{CH}(\text{NH}_2)\text{COOH} \cdot \text{HCl}$  (Aldrich 28,736-9); (12) 0-methyldopamine hydrochloride

$\text{CH}_3\text{OC}_6\text{H}_3(\text{OH})\text{CH}_2\text{CH}_2\text{NH}_2 \cdot \text{HCl}$  (Aldrich 19,596-0, Aldrich 16,431-3); (13) hydroxy dopamine hydrochloride  $(\text{HO})_3\text{C}_6\text{H}_2\text{CH}_2\text{CH}_2\text{NH}_2 \cdot \text{HCl}$  (Aldrich 15,156-4, 14,980-2); (14) hydroxy dopamine hydrobromide  $(\text{HO})_3\text{C}_6\text{H}_2\text{CH}_2\text{CH}_2\text{NH}_2 \cdot \text{HBr}$  (Aldrich 16,295-7); (15) 3-hydroxytyramine hydrochloride  $(\text{HO})_2\text{C}_6\text{H}_3\text{CH}_2\text{CH}_2\text{NH}_2 \cdot \text{HCl}$  (Aldrich H6,025-5); (16) 3-hydroxytyramine hydrobromide  $(\text{HO})_2\text{C}_6\text{H}_3\text{CH}_2\text{CH}_2\text{NH}_2 \cdot \text{HBr}$  (Aldrich 16,113-6); (17) o-benzyl hydroxyl amine hydrochloride  $\text{C}_6\text{H}_5\text{CH}_2\text{ONH}_2 \cdot \text{HCl}$  (Aldrich B2,298-4); (18) aminomethyl-1-cyclohexanol hydrochloride  $\text{H}_2\text{NCH}_2\text{C}_6\text{H}_{10}\text{OH} \cdot \text{HCl}$  (Aldrich 19,141-8); (19) 2-amino cyclohexanol hydrochloride  $\text{H}_2\text{NC}_6\text{H}_{10}\text{OH} \cdot \text{HCl}$  (Aldrich 26,376-1); (20) 4-amino-2,3-dimethyl phenol hydrochloride  $\text{H}_2\text{NC}_6\text{H}_2(\text{CH}_3)_2\text{OH} \cdot \text{HCl}$  (Aldrich 24,416-3); (21) 4-(2-hydroxyethylthio)1,3-phenylenediamine dihydrochloride  $\text{HO}(\text{CH}_2\text{CH}_2\text{S})\text{C}_6\text{H}_3(\text{NH}_2)_2 \cdot 2\text{HCl}$  (Aldrich 20,923-6); (22) 2-amino-3-hydroxy benzoic acid hydrochloride  $\text{HOC}_6\text{H}_3\text{NH}_2\text{COOH} \cdot \text{HCl}$  (Aldrich 30,690-8); (23) 4-hydroxy-3-methoxy benzyl amine hydrochloride  $\text{HOC}_6\text{H}_3(\text{OCH}_3)\text{CH}_2\text{NH}_2 \cdot \text{HCl}$  (Aldrich H3,660-5); (24) 4-amino phenol hydrochloride  $\text{H}_2\text{NC}_6\text{H}_4\text{OH} \cdot \text{HCl}$  (Aldrich 27,406-2); (25) 2-[2-(aminomethyl) phenyl thio] benzyl alcohol hydrochloride  $\text{H}_2\text{NCH}_2\text{C}_6\text{H}_4\text{SC}_6\text{H}_4\text{CH}_2\text{OH} \cdot \text{HCl}$  (Aldrich 34,632-2); (26) amino diphenyl methane hydrochloride  $(\text{C}_6\text{H}_5)_2\text{CHNH}_2 \cdot \text{HCl}$  (Aldrich 17,688-5); (27) (4-aminophenyl) trimethyl ammonium iodide hydrochloride  $(\text{CH}_3)_3\text{N}(\text{I})\text{C}_6\text{H}_4\text{NH}_2 \cdot \text{HCl}$  (Kodak 11372, available from Eastman Kodak Co.); (28) 4-aminoantipyrine hydrochloride (Kodak 6535, available from Eastman Kodak Co.), of the formula



and the like.

Also suitable are (VII) acid salts of aromatic amines having a hydrazine ( $-\text{NRNH}_2$ ) group, wherein R is hydrogen, alkyl, or aryl, such as (1) tolylhydrazine hydrochloride  $\text{CH}_3\text{C}_6\text{H}_4\text{NHNH}_2 \cdot \text{HCl}$  (Aldrich 28,190-5, T4,040-1, T4,060-6); (2) 3-chloro-p-tolyl hydrazine hydrochloride  $\text{ClC}_6\text{H}_3(\text{CH}_3)\text{NHNH}_2 \cdot \text{HCl}$  (Aldrich 15,343-5); (3) 4-chloro-o-tolylhydrazine hydrochloride  $\text{ClC}_6\text{H}_3(\text{CH}_3)\text{NHNH}_2 \cdot \text{HCl}$  (Aldrich 15,283-8); (4) chlorophenyl hydrazine hydrochloride  $\text{ClC}_6\text{H}_4\text{NHNH}_2 \cdot \text{HCl}$  (Aldrich 10,950-9; 15,396-6; C6,580-7); (5) 3-nitrophenyl hydrazine hydrochloride  $\text{O}_2\text{NC}_6\text{H}_4\text{NHNH}_2 \cdot \text{HCl}$  (Aldrich N2,180-4); (6) 4-isopropyl phenylhydrazine hydrochloride  $(\text{CH}_3)_2\text{CHC}_6\text{H}_4\text{NHNH}_2 \cdot \text{HCl}$  (Aldrich 32,431-0); (7) dimethyl phenyl hydrazine hydrochloride hydrate  $(\text{CH}_3)_2\text{C}_6\text{H}_3\text{NHNH}_2 \cdot \text{HCl} \cdot x\text{H}_2\text{O}$  (Aldrich 32,427-2, 32,428-0; 32,429-9); (8) 1,1-diphenyl hydrazine hydrochloride  $(\text{C}_6\text{H}_5)_2\text{NNH}_2 \cdot \text{HCl}$  (Aldrich 11,459-6); (9) 3-hydroxybenzyl hydrazine dihydrochloride  $\text{HOC}_6\text{H}_4\text{CH}_2\text{NHNH}_2 \cdot 2\text{HCl}$  (Aldrich 85,992-3); and the like.

Also suitable are (VIII) acid salts of aromatic diamine and substituted diamine containing compounds, such as (1) phenylene diamine dihydrochloride  $\text{C}_6\text{H}_4(\text{NH}_2)_2 \cdot 2\text{HCl}$  (Aldrich 3,590-3, 13,769-3); (2) N,N-dimethyl-1,3-phenylene diamine dihydrochloride  $(\text{CH}_3)_2\text{NC}_6\text{H}_4\text{NH}_2 \cdot 2\text{HCl}$  (Aldrich 21,922-3); (3) N,N-dimethyl-1,4-phenylene diamine monohydrochloride  $(\text{CH}_3)_2\text{NC}_6\text{H}_4\text{NH}_2 \cdot \text{HCl}$  (Aldrich 27,157-8); (4) N,N-dimethyl-1,4-phenylene diamine dihydrochloride  $(\text{CH}_3)_2\text{NC}_6\text{H}_4\text{NH}_2 \cdot 2\text{HCl}$  (Aldrich 21,923-1); (5) N,N-dimethyl-1,4-phenylene diamine sulfate  $(\text{CH}_3)_2\text{NC}_6\text{H}_4\text{NH}_2 \cdot \text{H}_2\text{SO}_4$  (Aldrich 18,638-4); (6) 4,4'-di-

amino diphenylamine sulfate ( $\text{H}_2\text{NC}_6\text{H}_4)_2\text{NH}\cdot\text{H}_2\text{SO}_4$  (Aldrich D1,620-7); (7) N,N-diethyl-1,4-phenylene diamine sulfate ( $\text{C}_2\text{H}_5)_2\text{NC}_6\text{H}_4\text{NH}_2\cdot\text{H}_2\text{SO}_4$  (Aldrich 16,834-3); (8) 2,4-diamino phenol dihydrochloride ( $\text{H}_2\text{N})_2\text{C}_6\text{H}_3\text{OH}\cdot\text{HCl}$  (Aldrich 23,010-3); (9) 4-(dimethyl amino) benzyl amine dihydrochloride ( $\text{CH}_3)_2\text{NC}_6\text{H}_4\text{CH}_2\text{NH}_2\cdot\text{HCl}$  (Aldrich 28,563-3); (10) 3,3'-dimethoxybenzidine hydrochloride hydrate  $[-\text{C}_6\text{H}_3(\text{OCH}_3)\text{NH}_2]_2\cdot\text{xHCl}\cdot\text{xH}_2\text{O}$  (Aldrich 19,124-8); (11) 4,4'-diaminostilbene dihydrochloride  $\text{H}_2\text{NC}_6\text{H}_4\text{CH}=\text{CHC}_6\text{H}_4\text{NH}_2\cdot\text{HCl}$  (Aldrich D2,520-6); (12) 4-(aminomethyl) benzene sulfonamide hydrochloride hydrate  $\text{H}_2\text{NCH}_2\text{C}_6\text{H}_4\text{SO}_2\text{NH}_2\cdot\text{HCl}\cdot\text{xH}_2\text{O}$  (Aldrich A6,180-2); (13) 4-methoxy-1,2-phenylene diamine dihydrochloride  $\text{CH}_3\text{OC}_6\text{H}_3(\text{NH}_2)_2\cdot\text{HCl}$  (Aldrich M2,040-4); (14) procaine hydrochloride  $\text{H}_2\text{NC}_6\text{H}_4\text{COOCH}_2\text{CH}_2\text{N}(\text{C}_2\text{H}_5)_2\cdot\text{HCl}$  (Aldrich 22,297-6); (15) procain amide hydrochloride  $\text{H}_2\text{NC}_6\text{H}_4\text{CONHCH}_2\text{CH}_2\text{N}(\text{C}_2\text{H}_5)_2\cdot\text{HCl}$  (Aldrich 22,296-8); (16) 3,3',5,5'-tetramethyl benzidine dihydrochloride hydrate  $[\text{C}_6\text{H}_2(\text{CH}_3)_2\text{-4-NH}_2]_2\cdot\text{HCl}\cdot\text{xH}_2\text{O}$  (Aldrich 86,151-0); (17) N-(1-naphthyl) ethylene diamine dihydrochloride  $\text{C}_{10}\text{H}_7\text{NHCH}_2\text{CH}_2\text{NH}_2\cdot\text{HCl}$  (Aldrich 22,248-8); (18) D,L-alanine-2-naphthylamide hydrochloride  $\text{CH}_3\text{CH}(\text{NH}_2)\text{CONHC}_{10}\text{H}_7\cdot\text{HCl}$  (Aldrich 85,677-0); (19) N-(4-methoxyphenyl)-1,4-phenylene diamine hydrochloride  $\text{CH}_3\text{OC}_6\text{H}_4\text{NHC}_6\text{H}_4\text{NH}_2\cdot\text{HCl}$  (Aldrich 21,702-6); (20) 2-methoxy-1,4-phenylene diamine sulfate hydrate  $\text{CH}_3\text{OC}_6\text{H}_3(\text{NH}_2)_2\cdot\text{H}_2\text{SO}_4\cdot\text{xH}_2\text{O}$  (Aldrich 17,006-2); (21) 2,2-dimethyl-1,3-propane diamine dihydrochloride  $\text{H}_2\text{NCH}_2\text{C}(\text{CH}_3)_2\text{CH}_2\text{NH}_2\cdot\text{HCl}$  (Aldrich 22,693-9); and the like.

Also suitable are (IX) acid salts of aromatic guanidine compounds, of the general formula  $\text{R}_8\text{-C}(\text{=NH})\text{NH}_2\text{H}_n\text{X}^{\text{n-}}$ , wherein  $\text{R}_8$  can be (but is not limited to) aryl (such as phenyl or the like), substituted aryl (such as amino phenyl, amido phenyl, or the like), arylalkyl (such as benzyl and the like), substituted arylalkyl (such as amino alkyl phenyl, mercaptyl benzyl, and the like) and the like,  $\text{X}$  is an anion, such as  $\text{Cl}^-$ ,  $\text{Br}^-$ ,  $\text{I}^-$ ,  $\text{HSO}_4^-$ ,  $\text{SO}_4^{2-}$ ,  $\text{NO}_3^-$ ,  $\text{HCOO}^-$ ,  $\text{CH}_3\text{COO}^-$ ,  $\text{HCO}_3^-$ ,  $\text{CO}_3^{2-}$ ,  $\text{H}_2\text{PO}_4^-$ ,  $\text{HPO}_4^{2-}$ ,  $\text{PO}_4^{3-}$ ,  $\text{SCN}^-$ ,  $\text{BF}_4^-$ ,  $\text{ClO}_4^-$ ,  $\text{SSO}_3^-$ ,  $\text{CH}_3\text{SO}_3^-$ , or the like, as well as mixtures thereof, and  $n$  is an integer of 1, 2, or 3, including (1) benzamidine hydrochloride  $\text{C}_6\text{H}_5\text{C}(\text{=NH})\text{NH}_2\cdot\text{HCl}$  (Kodak 6228, available from Eastman Kodak Co.) and benzamidine hydrochloride hydrate  $\text{C}_6\text{H}_5\text{C}(\text{=NH})\text{NH}_2\cdot\text{HCl}\cdot\text{xH}_2\text{O}$  (Aldrich B 200-4); (2) 4-amidino benzamide hydrochloride  $\text{H}_2\text{NC}(\text{=NH})\text{C}_6\text{H}_4\text{CONH}_2\cdot\text{HCl}$  (Aldrich 24,781-2); (3) 3-aminobenzamidine dihydrochloride  $\text{H}_2\text{NC}_6\text{H}_4\text{C}(\text{=NH})\text{NH}_2\cdot\text{HCl}$  (Aldrich 85,773-4); (4) 4-aminobenzamidine dihydrochloride  $\text{H}_2\text{NC}_6\text{H}_4\text{C}(\text{=NH})\text{NH}_2\cdot\text{HCl}$  (Aldrich 85,766-1); (5) 1-(3-phenyl propyl amino) guanidine hydrochloride  $\text{C}_6\text{H}_5(\text{CH}_2)_3\text{NHNH}(\text{=NH})\text{NH}_2\cdot\text{HCl}$  (Aldrich 22,161-9); (6) 2-benzyl-2-thiopseudourea hydrochloride  $\text{C}_6\text{H}_5\text{CH}_2\text{SC}(\text{=NH})\text{NH}_2\cdot\text{HCl}$  (Aldrich 25,103-8); and the like.

Also suitable are (X) acid salts of aromatic monoamines, such as those of the general formula  $\text{R}_9\text{-NH}_2\text{H}_n\text{X}^{\text{n-}}$ , wherein  $\text{R}_9$  can be (but is not limited to) aryl (such as phenyl or the like), substituted aryl (such as phenyl alkyl, phenyl cyclic alkyl, phenyl alkyl carbonyl halide, phenyl alkyl carbonyl halide, or the like), arylalkyl, substituted arylalkyl (such as alkoxy phenyl alkyl, aryloxy phenyl alkyl, aryloxy alkyl, or the like), or the like, and  $\text{X}$  is an anion, such as  $\text{Cl}^-$ ,  $\text{Br}^-$ ,  $\text{I}^-$ ,  $\text{HSO}_4^-$ ,  $\text{SO}_4^{2-}$ ,  $\text{NO}_3^-$ ,  $\text{HCOO}^-$ ,  $\text{CH}_3\text{COO}^-$ ,  $\text{HCO}_3^-$ ,  $\text{CO}_3^{2-}$ ,  $\text{H}_2\text{PO}_4^-$ ,  $\text{HPO}_4^{2-}$ ,  $\text{PO}_4^{3-}$ ,  $\text{SCN}^-$ ,  $\text{BF}_4^-$ ,  $\text{ClO}_4^-$ ,

$\text{SSO}_3^-$ ,  $\text{CH}_3\text{SO}_3^-$ ,  $\text{CH}_3\text{C}_6\text{H}_4\text{SO}_3^-$ , or the like, as well as mixtures thereof, and  $n$  is an integer of 1, 2, or 3, including (1) 2-phenyl cyclopropyl amine hydrochloride  $\text{C}_6\text{H}_5\text{C}_3\text{H}_4\text{NH}_2\cdot\text{HCl}$  (Aldrich P2,237-0); (2) amino diphenyl methane hydrochloride  $(\text{C}_6\text{H}_5)_2\text{CHNH}_2\cdot\text{HCl}$  (Aldrich 17,688-5); (3) (R)-(-)-2-phenyl glycine chloride hydrochloride  $\text{C}_6\text{H}_5\text{CH}(\text{NH}_2)\text{COCl}\cdot\text{HCl}$  (Aldrich 34,427-3); (4) phenethylamine hydrochloride  $\text{C}_6\text{H}_5(\text{CH}_2)_2\text{NH}_2\cdot\text{HCl}$  (Aldrich 25,041-4); (5) 2,4-dimethoxybenzylamine hydrochloride  $(\text{CH}_3\text{O})_2\text{C}_6\text{H}_3\text{CH}_2\text{NH}_2\cdot\text{HCl}$  (Aldrich 17,860-8); (6) 3,4-dibenzoyloxy phenethyl amine hydrochloride  $(\text{C}_6\text{H}_5\text{CH}_2\text{O})_2\text{C}_6\text{H}_3\text{CH}_2\text{CH}_2\text{NH}_2\cdot\text{HCl}$  (Aldrich 16,189-6); (7) 2,2-diphenyl propylamine hydrochloride  $\text{CH}_3\text{C}(\text{C}_6\text{H}_5)_2\text{CHNH}_2\cdot\text{HCl}$  (Aldrich 18,768-2); (8) 2,4,6-trimethoxy benzylamine hydrochloride  $(\text{CH}_3\text{O})_3\text{C}_6\text{H}_2\text{CH}_2\text{NH}_2\cdot\text{HCl}$  (Aldrich 30,098-5); (9) 4-benzoyloxyaniline hydrochloride  $\text{C}_6\text{H}_5\text{CH}_2\text{OC}_6\text{H}_4\text{NH}_2\cdot\text{HCl}$  (Aldrich 11,663-7); (10) benzylamine hydrochloride  $\text{C}_6\text{H}_5\text{CH}_2\text{NH}_2\cdot\text{HCl}$  (Aldrich 21,425-6); and the like.

Also suitable are (XI) acid salts of aromatic amino esters, such as (1) N- $\alpha$ -p-tosyl-L-arginine methylester hydrochloride

$\text{H}_2\text{NC}(\text{=NH})\text{NH}(\text{CH}_2)_3\text{CH}(\text{NSO}_2\text{C}_6\text{H}_4\text{CH}_3)\text{COOCH}_3\cdot\text{HCl}$  (Aldrich T4,350-8); (2) L-phenyl alanine methyl ester hydrochloride  $\text{C}_6\text{H}_5\text{CH}_2\text{CH}(\text{NH}_2)\text{COOCH}_3\cdot\text{HCl}$  (Aldrich P1,720-2); (3) D,L-4-chlorophenylalanine methyl ester hydrochloride  $\text{ClC}_6\text{H}_4\text{CH}_2\text{CH}(\text{NH}_2)\text{COOCH}_3\cdot\text{HCl}$  (Aldrich 27,181-0); (4) ethyl 4-aminobenzoate hydrochloride  $\text{H}_2\text{NC}_6\text{H}_4\text{COOC}_2\text{H}_5\cdot\text{HCl}$  (Aldrich 29,366-0); (5) L-phenyl alanine ethyl ester hydrochloride  $\text{C}_6\text{H}_5\text{CH}_2\text{CH}(\text{NH}_2)\text{COOC}_2\text{H}_5\cdot\text{HCl}$  (Aldrich 22,070-1); (6) D,L-4-chlorophenylalanine ethyl ester hydrochloride  $\text{ClC}_6\text{H}_4\text{CH}_2\text{CH}(\text{NH}_2)\text{COOC}_2\text{H}_5\cdot\text{HCl}$  (Aldrich 15,678-7); and the like.

Also suitable are (XII) acid salts of aromatic imines, such as (1) ephedrine hydrochloride  $\text{C}_6\text{H}_5\text{CH}[\text{CH}(\text{NHCH}_3)\text{CH}_3]\text{OH}\cdot\text{HCl}$  (Aldrich 28,574-9; 86,223-1); (2) ephedrine nitrate  $\text{C}_6\text{H}_5\text{CH}[\text{CH}(\text{NHCH}_3)\text{CH}_3]\text{OH}\cdot\text{HNO}_3$  (Aldrich 86,039-5); (3) (1S, 2S)-(+)-pseudoephedrine hydrochloride  $\text{C}_6\text{H}_5\text{CH}[\text{CH}(\text{NHCH}_3)\text{CH}_3]\text{OH}\cdot\text{HCl}$  (Aldrich 29,461-6); (4) (±) 4-hydroxyephedrine hydrochloride  $\text{HOC}_6\text{H}_4\text{CH}(\text{OH})\text{CH}(\text{CH}_3)\text{NHCH}_3\cdot\text{HCl}$  (Aldrich 10,615-1); (5) (±)-isoproterenol hydrochloride 3,4-( $\text{HO})_2\text{C}_6\text{H}_3\text{CH}(\text{OH})\text{CH}_2\text{NHCH}(\text{CH}_3)_2\cdot\text{HCl}$  (Aldrich 1-2, 790-2); (6) (±)-propranolol hydrochloride  $\text{C}_{10}\text{H}_7\text{OCH}_2\text{CH}(\text{OH})\text{CH}_2\text{NHCH}(\text{CH}_3)_2\cdot\text{HCl}$  (Aldrich 22,298-4); (7) chlorohexidine diacetate hydrate  $[-(\text{CH}_2)_3\text{NHC}(\text{=NH})\text{NHC}(\text{=NH})\text{NHC}_6\text{H}_4\text{Cl}]_2\cdot 2\text{CH}_3\text{COOH}\cdot\text{xH}_2\text{O}$  (Aldrich 23,386-2); (8) (±)-2-(methyl amino) propiophenone hydrochloride  $\text{C}_6\text{H}_5\text{COCH}(\text{CH}_3)\text{NHCH}_3\cdot\text{HCl}$  (Aldrich 31,117-0); (9) 4-methyl aminophenol sulfate  $(\text{CH}_3\text{NHC}_6\text{H}_4\text{OH})_2\cdot\text{H}_2\text{SO}_4$  (Aldrich 32,001-3); (10) methyl benzimidate hydrochloride  $\text{C}_6\text{H}_5\text{C}(\text{=NH})\text{OCH}_3\cdot\text{HCl}$  (Aldrich 22,051-5); (11) (±)-methanephrine hydrochloride  $\text{HOC}_6\text{H}_3(\text{OCH}_3)\text{CH}(\text{CH}_2\text{NHCH}_3)\text{OH}\cdot\text{HCl}$  (Aldrich 27,428-3); (12) malonaldehyde bis (phenyl imine) dihydrochloride  $\text{CH}_2(\text{CH}=\text{NC}_6\text{H}_5)_2\cdot\text{HCl}$  (Aldrich 34,114-2); (13) (±)-ketamine hydrochloride  $\text{C}_1\text{C}_6\text{H}_4\text{C}_6\text{H}_8(\text{=O})\text{NHCH}_3\cdot\text{HCl}$  (Aldrich 34,309-9); (14) (±)-isoproterenol sulfate dihydrate [3,4-( $\text{HO})_2\text{C}_6\text{H}_3\text{CH}(\text{OH})\text{CH}_2\text{NH}(\text{CH}_3)_2]_2\cdot\text{H}_2\text{SO}_4\cdot 2\text{H}_2\text{O}$  (Aldrich 10,044-7); (15) isoproterenol L-bitartrate 3,4-( $\text{HO})_2\text{C}_6\text{H}_3\text{CH}(\text{OH})\text{CH}_2\text{NH}(\text{CH}_3)_2\cdot \text{HOOC-CH}(\text{OH})\text{CH}_2\text{COOH}$  (Aldrich 18,881-6); (16) diphenyhydramine hydrochloride  $(\text{C}_6\text{H}_5)_2\text{CHOCH}_2\text{CH}_2\text{N}(\text{CH}_3)_2\cdot\text{HCl}$  (Aldrich 28,566-8);

- (17) 3-dimethylamino propiophenone hydrochloride  $C_6H_5COCH_2CH_2N(CH_3)_2 \cdot HCl$  (Aldrich D14,480-0); (18) neostigmine bromide 3-[ $(CH_3)_2NCOO$ ] $C_6H_4N(CH_3)_2Br$  (Aldrich 28,679-6); (19) neostigmine methyl sulfate 3-[ $(CH_3)_2NCOO$ ] $C_6H_4N(CH_3)_3(OSO_3CH_3)$  (Aldrich 28,681-8); (20) orphenadrine hydrochloride  $CH_3C_6H_4CH(C_6H_5)OCH_2CH_2N(CH_3)_2 \cdot HCl$  (Aldrich 13,128-8); and the like.

Examples of suitable quaternary choline halides include (1) choline chloride [(2-hydroxyethyl) trimethyl ammonium chloride]  $HOCH_2CH_2N(CH_3)_3Cl$  (Aldrich 23,994-1) and choline iodide  $HOCH_2CH_2N(CH_3)_3I$  (Aldrich C7,971-9); (2) acetyl choline chloride  $CH_3COOCH_2CH_2N(CH_3)_3Cl$  (Aldrich 13,535-6), acetyl choline bromide  $CH_3COOCH_2CH_2N(CH_3)_3Br$  (Aldrich 85,968-0), and acetyl choline iodide  $CH_3COOCH_2CH_2N(CH_3)_3I$  (Aldrich 10,043-9); (3) acetyl- $\beta$ -methyl choline chloride  $CH_3COOCH(CH_3)CH_2N(CH_3)Cl$  (Aldrich A1,800-1) and acetyl- $\beta$ -methyl choline bromide  $CH_3COOCH(CH_3)CH_2N(CH_3)_3Br$  (Aldrich 85,554-5); (4) benzoyl choline chloride  $C_6H_5COOCH_2CH_2N(CH_3)_3Cl$  (Aldrich 21,697-6); (5) carbamyl choline chloride  $H_2NCOOCH_2CH_2N(CH_3)_3Cl$  (Aldrich C240-9); (6) D,L-carnitinamide hydrochloride  $H_2NCOCH_2CH(OH)CH_2N(CH_3)_3Cl$  (Aldrich 24,783-9); (7) D,L-carnitine hydrochloride  $HOOCCH_2CH(OH)CH_2N(CH_3)_3Cl$  (Aldrich C1,600-8); (8) (2-bromo ethyl) trimethyl ammonium chloride [bromo choline chloride]  $BrCH_2CH_2N(CH_3)_3Br$  (Aldrich 11,719-6); (9) (2-chloro ethyl) trimethyl ammonium chloride [chloro choline chloride]  $ClCH_2CH_2N(CH_3)_3Cl$  (Aldrich 23,443-5); (10) (3-carboxy propyl) trimethyl ammonium chloride  $HOOC(CH_2)_3N(CH_3)_3Cl$  (Aldrich 26,365-6); (11) butyryl choline chloride  $CH_3CH_2CH_2COOCH_2CH_2N(CH_3)_3Cl$  (Aldrich 85,537-5); (12) butyryl thiocholine iodide  $CH_3CH_2CH_2COSCH_2CH_2N(CH_3)_3I$  (Aldrich B10,425-6); (13) S-propionyl thiocholine iodide  $C_2H_5COSCH_2CH_2N(CH_3)_3I$  (Aldrich 10,412-4); (14) S-acetylthiocholine bromide  $CH_3COSCH_2CH_2N(CH_3)_3Br$  (Aldrich 85,533-2) and S-acetylthiocholine iodide  $CH_3COSCH_2CH_2N(CH_3)_3I$  (Aldrich A2,230-0); (15) suberyl dicholine dichloride  $[-(CH_2)_3COOCH_2CH_2N(CH_3)_3Cl]_2$  (Aldrich 86,204-5) and suberyl dicholine diiodide  $[-(CH_2)_3COOCH_2CH_2N(CH_3)_3I]_2$  (Aldrich 86,211-8); and the like, as well as mixtures thereof.

Also suitable as antistatic agents are pyrrole and pyrrolidine acid salt compounds, of the general formulae



wherein  $R_1$ ,  $R_2$ ,  $R_3$ ,  $R_4$ ,  $R_5$ ,  $R_6$ ,  $R_7$ ,  $R_8$ , and  $R_9$  each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably

with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of  $R_1$ ,  $R_2$ ,  $R_3$ ,  $R_4$ ,  $R_5$ ,  $R_6$ ,  $R_7$ ,  $R_8$ , and  $R_9$  can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula  $xH_nY_n^-$ , wherein  $n$  is an integer of 1, 2, or 3,  $x$  is a number indicating the relative ratio between compound and acid (and may be a fraction), and  $Y$  is an anion, such as  $Cl^-$ ,  $Br^-$ ,  $I^-$ ,  $HSO_4^-$ ,  $SO_4^{2-}$ ,  $NO_3^-$ ,  $HCOO^-$ ,  $CH_3COO^-$ ,  $HCO_3^-$ ,  $CO_3^{2-}$ ,  $H_2PO_4^-$ ,  $HPO_4^{2-}$ ,  $PO_4^{3-}$ ,  $SCN^-$ ,  $BF_4^-$ ,  $ClO_4^-$ ,  $SSO_3^-$ ,  $CH_3SO_3^-$ ,  $CH_3C_6H_4SO_3^-$ ,  $SO_3^{2-}$ ,  $BrO_3^-$ ,  $IO_3^-$ ,  $ClO_3^-$ , or the like. Examples of suitable pyrrole and pyrrolidine acid salt compounds include (1) 1-amino pyrrolidine hydrochloride (Aldrich 12,310-2), of the formula:



(2) 2-(2-chloroethyl)-1-methyl pyrrolidine hydrochloride (Aldrich 13,952-1), of the formula:



37

(3) 1-(2-chloroethyl) pyrrolidine hydrochloride (Aldrich C4,280-7), of the formula:



(4) L-proline methyl ester hydrochloride (Aldrich 28,706-7), of the formula:



5

38

(8) 1-(4-chlorobenzyl)-2-(1-pyrrolidinyl methyl) benzimidazole hydrochloride (Aldrich 34,208-4), of the formula:



15

(9) biliverdin dihydrochloride (Aldrich 25,824-5), of the formula:



and the like.

Also suitable as antistatic agents are pyridine acid salt compounds, of the general formula

35



(5) tremarine dihydrochloride [1,1'-(2-butynylene) dipyrrolidine hydrochloride] (Aldrich T4,365-6), of the formula:



45

(6) ammonium pyrrolidine dithiocarbamate (Aldrich 14,269-7), of the formula:



50

(7) pyrrolidone hydrotribromide (Aldrich 15,520-9), of the formula:



55

wherein R<sub>1</sub>, R<sub>2</sub>, R<sub>3</sub>, R<sub>4</sub>, and R<sub>5</sub> s each, independently from one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R<sub>1</sub>, R<sub>2</sub>, R<sub>3</sub>, R<sub>4</sub>, and R<sub>5</sub>

60

65

can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula  $xH_nY_n^-$ , wherein n is an integer of 1, 2, or 3, x is a number indicating the relative ratio between compound and acid (and may be a fraction), and Y is an anion, such as  $Cl^-$ ,  $Br^-$ ,  $I^-$ ,  $HSO_4^-$ ,  $SO_4^{2-}$ ,  $NO_3^-$ ,  $HCOO^-$ ,  $CH_3COO^-$ ,  $HCO_3^-$ ,  $CO_3^{2-}$ ,  $H_2PO_4^-$ ,  $HPO_4^{2-}$ ,  $PO_4^{3-}$ ,  $SCN^-$ ,  $BF_4^-$ ,  $ClO_4^-$ ,  $SSO_3^-$ ,  $CH_3SO_3^-$ ,  $CH_3C_6H_4SO_3^-$ ,  $SO_3^{2-}$ ,  $BrO_3^-$ ,  $IO_3^-$ ,  $ClO_3^-$ , or the like. Examples of suitable pyridine acid salt compounds include

(1) pyridine hydrobromide (Aldrich 30,747-5), of the formula:



(2) pyridine hydrochloride (Aldrich 24,308-6), of the formula:



(3) 2-(chloromethyl) pyridine hydrochloride (Aldrich 16,270-1), of the formula:



(4) 2-pyridylacetic acid hydrochloride (Aldrich P6,560-6), of the formula:



(5) nicotinoyl chloride hydrochloride (Aldrich 21,338-1), of the formula:



(6) 2-hydrazinopyridine dihydrochloride (Aldrich H1,710-4), of the formula:



(7) 2-(2-methyl aminoethyl) pyridine dihydrochloride (Aldrich 15,517-9), of the formula:



(8) 1-methyl-1,2,3,6-tetrahydropyridine hydrochloride (Aldrich 33,238-0), of the formula:



(9) 2,6-dihydroxypyridine hydrochloride (Aldrich D12,000-6), of the formula:



(10) 3-hydroxy-2(hydroxymethyl) pyridine hydrochloride (Aldrich H3,153-0), of the formula:



(11) pyridoxine hydrochloride (Aldrich 11,280-1), of the formula:



(12) pyridoxal hydrochloride (Aldrich 27,174-8), of the formula:



(13) pyridoxal 5-phosphate monohydrate (Aldrich 85,786-6), of the formula:



(14) 3-amino-2,6-dimethoxy pyridine hydrochloride (Aldrich 14,325-1), of the formula:



(15) pyridoxamine dihydrochloride monohydrate (Aldrich 28,709-1), of the formula:



(16) iproniazid phosphate (isonicotinic acid 2-isopropyl hydrazide phosphate) (Aldrich I-1,265-4), of the formula:



(17) trielennamine hydrochloride (Aldrich 28,738-5), of the formula:



and the like.

Also suitable as antistatic agents are piperidine and homopiperidine acid salt compounds, of the general formulae



-continued



wherein R<sub>1</sub>, R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>10</sub>, R<sub>11</sub>, R<sub>12</sub>, R<sub>13</sub>, R<sub>14</sub>, and R<sub>15</sub> each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R<sub>1</sub>, R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>10</sub>, R<sub>11</sub>, R<sub>12</sub>, R<sub>13</sub>, R<sub>14</sub>, and R<sub>15</sub> can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula xH<sub>n</sub>Y<sub>n</sub><sup>-</sup>, wherein n is an integer of 1, 2, or 3, x is a number indicating the relative ratio between compound and acid (and may be a fraction), and Y is an anion, such as Cl<sup>-</sup>, Br<sup>-</sup>, I<sup>-</sup>, HSO<sub>4</sub><sup>2-</sup>, SO<sub>4</sub><sup>2-</sup>, NO<sub>3</sub><sup>-</sup>,

43

$\text{HCOO}^-$ ,  $\text{CH}_3\text{COO}^-$ ,  $\text{HCO}_3^-$ ,  $\text{CO}_3^{2-}$ ,  $\text{H}_2\text{PO}_4^-$ ,  $\text{HPO}_4^{2-}$ ,  $\text{PO}_4^{3-}$ ,  $\text{SCN}^-$ ,  $\text{BF}_4^-$ ,  $\text{ClO}_4^-$ ,  $\text{SSO}_3^-$ ,  $\text{CH}_3\text{SO}_3^-$ ,  $\text{CH}_3\text{C}_6\text{H}_4\text{SO}_3^-$ ,  $\text{SO}_3^{2-}$ ,  $\text{BrO}_3^-$ ,  $\text{IO}_3^-$ ,  $\text{ClO}_3^-$ , or the like. Examples of suitable piperidine and homopiperidine acid salts include

(1) 2-(hexamethylene imino) ethyl chloride monohydrochloride (Aldrich H1,065-7), of the formula:



(2) 3-(hexahydro-1H-azepin-1-yl)-3'-nitropropiophenone hydrochloride (Aldrich 15,912-3), of the formula:



(3) imipramine hydrochloride [5-(3-dimethyl aminopropyl)-10,11-dihydro 5H-dibenzo-(b,f) azepine hydrochloride] (Aldrich 28,626-5), of the formula:



(4) carbamezepine [5H-dibenzo (b,f)-azepine-5-carboxamide] (Aldrich 30,948-6), of the formula:



(5) 5,6,11,12-tetrahydro dibenz [b,f] azocine hydrochloride (Aldrich 18,761-5), of the formula:



44

(6) 2-iminopiperidine hydrochloride (Aldrich 13,117-2), of the formula:



10 and the like.

Also suitable as antistatic agents are quinoline and isoquinoline acid salt compounds, of the general formulae:



wherein  $R_1$ ,  $R_2$ ,  $R_3$ ,  $R_4$ ,  $R_5$ ,  $R_6$ , and  $R_7$  each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of  $R_1$ ,  $R_2$ ,  $R_3$ ,  $R_4$ ,  $R_5$ ,  $R_6$ ,  $R_7$ ,  $R_8$ , and  $R_9$  can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the

like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula  $xH_nY_n^-$ , wherein  $n$  is an integer of 1, 2, or 3,  $x$  is a number indicating the relative ratio between compound and acid (and may be a fraction), and  $Y$  is an anion, such as  $Cl^-$ ,  $Br^-$ ,  $I^-$ ,  $HSO_4^-$ ,  $SO_4^{2-}$ ,  $NO_3^-$ ,  $HCOO^-$ ,  $CH_3COO^-$ ,  $HCO_3^-$ ,  $CO_3^{2-}$ ,  $H_2PO_4^-$ ,  $HPO_4^{2-}$ ,  $PO_4^{3-}$ ,  $SCN^-$ ,  $BF_4^-$ ,  $ClO_4^-$ ,  $SSO_3^-$ ,  $CH_3SO_3^-$ ,  $CH_3C_6H_4SO_3^-$ ,  $SO_3^{2-}$ ,  $BrO_3^-$ ,  $IO_3^-$ ,  $ClO_3^-$ , or the like. Examples of suitable quinoline and isoquinoline acid salt compounds include

(1) 8-hydroxyquinoline hemisulfate hemihydrate (Aldrich 10,807-3), of the formula:



(2) 5-amino-8-hydroxy quinoline dihydrochloride (Aldrich 30,552-9), of the formula:



(3) 2-(chloromethyl) quinoline monohydrochloride (Aldrich C5,710-3), of the formula:



(4) 8-hydroxyquinoline-5-sulfonic acid monohydrate (Aldrich H5,875-7), of the formula:



(5) 8-ethoxy-5-quinoline sulfonic acid sodium salt hydrate (Aldrich 17,346-0), of the formula:



(6) 1,2,3,4-tetrahydroisoquinoline hydrochloride (Aldrich 30,754-8), of the formula:



(7) 1,2,3,4-tetrahydro-3-isoquinoline carboxylic acid hydrochloride (Aldrich 21,493-0), of the formula:



(8) 6,7-dimethoxy-1,2,3,4-tetrahydro isoquinoline hydrochloride (Aldrich 29,191-9), of the formula:



(9) 1-methyl-6,7-dihydroxy-1,2,3,4-tetrahydro isoquinoline hydrobromide (Aldrich 24,420-1), of the formula:



(10) primaquine diphosphate [8-(4-amino-1-methyl butyl amino)-6-methoxy quinoline diphosphate] (Aldrich 16,039-3), of the formula:



(11) pentaquine phosphate (Aldrich 30,207-4), of the formula:



(12) dibucaine hydrochloride [2-butoxy-N-(2-diethyl amino ethyl)-4-quinoline carboxamide hydrochloride] (Aldrich 28,555-2), of the formula:



(13) 9-aminoacridine hydrochloride hemihydrate (Aldrich A3,840-1), of the formula:



(14) 3,6-diamino acridine hemisulfate (Aldrich 19,822-6), of the formula:



(15) 2-quinoline thiol hydrochloride (Aldrich 35,978-5), of the formula:



(16) (-) sparteine sulfate pentahydrate (Aldrich 23,466-4), of the formula:



(17) papaverine hydrochloride (Aldrich 22,287-9), of the formula:



(18) (+)-emetine dihydrochloride hydrate (Aldrich 21,928-2), of the formula:



(19) 1,10-phenanthroline monohydrochloride monohydrate (Aldrich P1,300-2), of the formula:



(20) neocuproine hydrochloride trihydrate (Aldrich 12,189-6), of the formula:



and the like.

Also suitable as antistatic agents are quinuclidine acid salt compounds, of the general formula



wherein R<sub>1</sub>, R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>10</sub>, R<sub>11</sub>, and R<sub>12</sub> each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R<sub>1</sub>, R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>10</sub>, R<sub>11</sub>, and R<sub>12</sub> can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups,

49

amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula  $xH_nY_n^-$ , wherein n is an integer of 1, 2, or 3, x is a number indicating the relative ratio between compound and acid (and may be a fraction), and Y is an anion, such as  $Cl^-$ ,  $Br^-$ ,  $I^-$ ,  $HSO_4^-$ ,  $SO_4^{2-}$ ,  $NO_3^-$ ,  $HCOO^-$ ,  $CH_3COO^-$ ,  $HCO_3^-$ ,  $CO_3^{2-}$ ,  $H_2PO_4^-$ ,  $HPO_4^{2-}$ ,  $PO_4^{3-}$ ,  $SCN^-$ ,  $BF_4^-$ ,  $ClO_4^-$ ,  $SSO_3^-$ ,  $CH_3SO_3^-$ ,  $CH_3C_6H_5SO_3^-$ ,  $SO_3^{2-}$ ,  $BrO_3^-$ ,  $IO_3^-$ ,  $ClO_3^-$ , or the like. Examples of suitable quinuclidine acid salt compounds include

(1) quinuclidine hydrochloride (Aldrich 13,591-7), of the formula:



(2) 3-quinuclidinol hydrochloride (Aldrich Q188-3), of the formula:



(3) 3-quinuclidinone hydrochloride (Aldrich Q190-5), of the formula:



(4) 2-methylene-3-quinuclidinone dihydrate hydrochloride (Aldrich M4,612-8), of the formula:



(5) 3-amino quinuclidine dihydrochloride (Aldrich 10,035-8), of the formula:



(6) 3-chloro quinuclidine hydrochloride (Aldrich 12,521-0), of the formula:



50

(7) quinidine sulfate dihydrate (Aldrich 14,589-0), of the formula:



(8) quinine monohydrochloride dihydrate (Aldrich 14,592-0), of the formula:



(9) quinine sulfate monohydrate (Aldrich 14,591-2), of the formula:



(10) hydroquinidine hydrochloride (Aldrich 25,481-9), of the formula:



51

(11) hydroquinine hydrobromide dihydrate (Aldrich 34,132-0), of the formula:



and the like.

Also suitable as antistatic agents are indole and indazole acid salt compounds, of the general formulae



52

groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula  $xH_nY_n^-$ , wherein n is an integer of 1, 2, or 3, x is a number indicating the relative ratio between compound and acid (and may be a fraction), and  $Y^-$  is an anion, such as  $Cl^-$ ,  $Br^-$ ,  $I^-$ ,  $HSO_4^-$ ,  $SO_4^{2-}$ ,  $NO_3^-$ ,  $HCOO^-$ ,  $CH_3COO^-$ ,  $HCO_3^-$ ,  $CO_3^{2-}$ ,  $H_2PO_4^-$ ,  $HPO_4^{2-}$ ,  $PO_4^{3-}$ ,  $SCN^-$ ,  $BF_4^-$ ,  $ClO_4^-$ ,  $SSO_3^-$ ,  $CH_3SO_3^-$ ,  $CH_3C_6H_4SO_3^-$ ,  $SO_3^{2-}$ ,  $BrO_3^-$ ,  $IO_3^-$ ,  $ClO_3^-$ , or the like. Examples of suitable indole and indazole acid salt compounds include

(1) tryptamine hydrochloride (Aldrich 13,224-1), of the formula:



<sup>30</sup> (2) 5-methyl tryptamine hydrochloride (Aldrich 13,422-8),  
of the formula:



(3) serotonin hydrochloride hemihydrate (5-hydroxy tryptamine hydrochloride hemihydrate) (Aldrich 23,390-0) of the formula:



50 (4) norharman hydrochloride monohydrate (Aldrich 28,687-7), of the formula:



(5) harmane hydrochloride monohydrate (Aldrich 25,051-1), of the formula:



53

(6) harmine hydrochloride hydrate (Aldrich 12,848-1), of the formula:



(7) harmaline hydrochloride dihydrate (Aldrich H10-9), of the formula:



(8) harmol hydrochloride dihydrate (Aldrich 11,655-6), of the formula:



(9) harmalol hydrochloride dihydrate (Aldrich H12-5), of the formula:



(10) 3,6-diamino acridine hydrochloride (Aldrich 13,110-5), of the formula:



(11) S-(3-indolyl)isothiuronium iodide (Aldrich 16,097-0), of the formula:



54

(12) yohimbine hydrochloride (Aldrich Y20-8), of the formula:



(13) 4,5-dihydro-3-(4-pyridinyl)-2H-benz[g] indazole methane sulfonate (Aldrich 21,413-2), of the formula:



and the like.

Also suitable as antistatic agents are pyrimidine acid salt compounds, of the general formula



wherein R<sub>1</sub>, R<sub>2</sub>, R<sub>3</sub>, and R<sub>4</sub> each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto

groups, nitroso groups, halogen atoms, nitro groups, sulfone groups, acyl groups, acid anhydride groups, azide groups, and the like, wherein two or more of R<sub>1</sub>, R<sub>2</sub>, R<sub>3</sub>, R<sub>4</sub>, R<sub>5</sub>, R<sub>6</sub>, R<sub>7</sub>, R<sub>8</sub>, and R<sub>9</sub> can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula xH<sub>n</sub>Y<sub>n</sub><sup>-</sup>, wherein n is an integer of 1, 2, or 3, x is a number indicating the relative ratio between compound and acid (and may be a fraction), and Y is an anion, such as Cl<sup>-</sup>, Br<sup>-</sup>, I<sup>-</sup>, HSO<sub>4</sub><sup>2-</sup>, SO<sub>4</sub><sup>2-</sup>, NO<sub>3</sub><sup>-</sup>, HCOO<sup>-</sup>, CH<sub>3</sub>COO<sup>-</sup>, HCO<sub>3</sub><sup>-</sup>, CO<sub>3</sub><sup>2-</sup>, H<sub>2</sub>PO<sub>4</sub><sup>-</sup>, HPO<sub>4</sub><sup>2-</sup>, PO<sub>4</sub><sup>3-</sup>, SCN<sup>-</sup>, BF<sub>4</sub><sup>-</sup>, ClO<sub>4</sub><sup>-</sup>, SSO<sub>3</sub><sup>-</sup>, CH<sub>3</sub>SO<sub>3</sub><sup>-</sup>, CH<sub>3</sub>C<sub>6</sub>H<sub>4</sub>SO<sub>3</sub><sup>-</sup>, SO<sub>3</sub><sup>2-</sup>, BrO<sub>3</sub><sup>-</sup>, IO<sub>3</sub><sup>-</sup>, ClO<sub>3</sub><sup>-</sup>, or the like. Examples of suitable pyrimidine acid salt compounds include

(1) 2-hydroxypyrimidine hydrochloride (Aldrich H5,740-8), of the formula:



(2) 2-hydroxy-4-methyl pyrimidine hydrochloride (Aldrich H4,320-2), of the formula:



(3) 4,6-dimethyl-2-hydroxypyrimidine hydrochloride (Aldrich 33,996-2), of the formula:



(4) 2-mercaptop-4-methyl pyrimidine hydrochloride (Aldrich M480-5), of the formula:



(5) 4,6-diamino pyrimidine hemisulfate monohydrate (Aldrich D2,480-3), of the formula:



(6) 4,5,6-triamino pyrimidine sulfate hydrate (Aldrich T4,600-0; 30,718-1), of the formula:



(7) 4,5-diamino-6-hydroxy pyrimidine sulfate (Aldrich D1,930-3), of the formula:



(8) 2,4-diamino-6-mercaptop pyrimidine hemisulfate (Aldrich D1,996-6), of the formula:



(9) 2,4-diamino-6-hydroxy pyrimidine hemisulfate hydrate (Aldrich 30,231-7), of the formula:



(10) 6-hydroxy-2,4,5-triamino pyrimidine sulfate (Aldrich H5,920-6), of the formula:



(11) 5,6-diamino-2,4-dihydroxy pyrimidine sulfate (Aldrich D1,510-3), of the formula:



(12)  $N^4$ -(2-amino-4-pyrimidinyl) sulfanilamide monohydrochloride (Aldrich 15,237-4), of the formula:



(13) 4,5,6-triamino-2(1H)-pyrimidinethione sulfate (Aldrich 26,096-7), of the formula:



(14) 2,4,5,6-tetraamino pyrimidine sulfate (Aldrich T380-7), of the formula:



(15) (-)-cyclocytidine hydrochloride (Aldrich 85,883-8), of the formula:



(16) cytosine arabinoside hydrochloride (Aldrich 85,585-5), of the formula:



and the like.

Also suitable as antistatic agents are pyrazole acid salt compounds, of the general formula



10 wherein  $R_1$ ,  $R_2$ ,  $R_3$ , and  $R_4$  each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of  $R_1$ ,  $R_2$ ,  $R_3$ ,  $R_4$ ,  $R_5$ ,  $R_6$ ,  $R_7$ ,  $R_8$ , and  $R_9$  can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula  $xH_nY_n^-$ , wherein  $n$  is an integer of 1, 2, or 3,  $x$  is a number indicating the relative ratio between compound and acid (and may be a fraction), and  $Y$  is an anion, such as  $Cl^-$ ,  $Br^-$ ,  $I^-$ ,  $HSO_4^-$ ,  $SO_4^{2-}$ ,  $NO_3^-$ ,  $HCOO^-$ ,  $CH_3COO^-$ ,  $HCO_3^-$ ,  $CO_3^{2-}$ ,  $H_2PO_4^-$ ,  $HPO_4^{2-}$ ,  $PO_4^{3-}$ ,  $SCN^-$ ,  $BF_4^-$ ,  $ClO_4^-$ ,  $SSO_3^-$ ,  $CH_3SO_3^-$ ,  $CH_3C_6H_4SO_3^-$ ,  $SO_3^{2-}$ ,  $BrO_3^-$ ,  $IO_3^-$ ,  $ClO_3^-$ , or the like. Examples of suitable pyrazole acid salt compounds include

(1) 4-methyl pyrazole hydrochloride (Aldrich 28,667-2)



(2) 3,4-diamino-5-hydroxy pyrazole sulfate (Aldrich D1,900-1)



(3) (3,5-dimethyl pyrazole-1-carboxamidine nitrate) (Aldrich D18,225-7)



(4) 3-amino-4-pyrazole carboxamide hemisulfate (Aldrich 15,305-2)



(5) acid salt of 6-amino indazole hydrochloride (Aldrich A5,955-7)



and the like.

Also suitable as antistatic agents are oxazole and isoxazole acid salt compounds, of the general formulae



-continued



wherein R<sub>1</sub>, R<sub>2</sub>, R<sub>3</sub>, and R<sub>4</sub> each, independently of one another, can be (but are not limited to) hydrogen atoms, alkyl groups, preferably with from 1 to about 6 carbon atoms, and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R<sub>1</sub>, R<sub>2</sub>, R<sub>3</sub>, R<sub>4</sub>, R<sub>5</sub>, R<sub>6</sub>, R<sub>7</sub>, R<sub>8</sub>, and R<sub>9</sub> can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula xH<sub>n</sub>Y<sub>n</sub><sup>-</sup>, wherein n is an integer of 1, 2, or 3, x is a number indicating the relative ratio between compound and acid (and may be a fraction), and Y is an anion, such as Cl<sup>-</sup>, Br<sup>-</sup>, I<sup>-</sup>, HSO<sub>4</sub><sup>2-</sup>, SO<sub>4</sub><sup>2-</sup>, NO<sub>3</sub><sup>-</sup>, HCOO<sup>-</sup>, CH<sub>3</sub>COO<sup>-</sup>, HCO<sub>3</sub><sup>-</sup>, CO<sub>3</sub><sup>2-</sup>, H<sub>2</sub>PO<sub>4</sub><sup>-</sup>, HPO<sub>4</sub><sup>2-</sup>, PO<sub>4</sub><sup>3-</sup>, SCN<sup>-</sup>, BF<sub>4</sub><sup>-</sup>, ClO<sub>4</sub><sup>-</sup>, SSO<sub>3</sub><sup>-</sup>, CH<sub>3</sub>SO<sub>3</sub><sup>-</sup>, CH<sub>3</sub>C<sub>6</sub>H<sub>4</sub>SO<sub>3</sub><sup>-</sup>, SO<sub>3</sub><sup>2-</sup>, BrO<sub>3</sub><sup>-</sup>, IO<sub>3</sub><sup>-</sup>, ClO<sub>3</sub><sup>-</sup>, or the like. Examples of suitable oxazole and isoxazole acid salt compounds include

61

(1) 3,3'-dimethyl oxacarbocyanine iodide (Aldrich 32,069-2), of the formula:



(2) 2-ethyl-5-phenyl isoxazolium-3'-sulfonate (Aldrich E4,526-0), of the formula:



(3) 2-chloro-3-ethylbenzoxazolium tetrafluoroborate (Aldrich 23,255-6), of the formula:



(4) 2-tert-butyl-5-methyl isoxazolium perchlorate (Aldrich B9,695-3), of the formula:



(5) 5-phenyl-2-(4-pyridyl) oxazole hydrochloride hydrate (Aldrich 23,748-5), of the formula:



(6) 5-phenyl-2-(4-pyridyl) oxazole methyl tosylate salt (Aldrich 23,749-3), of the formula:



and the like.

Also suitable as antistatic agents are morpholine acid salt compounds, of the general formula



62

wherein R<sub>1</sub>, R<sub>2</sub>, R<sub>3</sub>, R<sub>4</sub>, R<sub>5</sub>, R<sub>6</sub>, R<sub>7</sub>, R<sub>8</sub>, and R<sub>9</sub> each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R<sub>1</sub>, R<sub>2</sub>, R<sub>3</sub>, R<sub>4</sub>, R<sub>5</sub>, R<sub>6</sub>, R<sub>7</sub>, R<sub>8</sub>, and R<sub>9</sub> can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula xH<sub>n</sub>Y<sub>n</sub><sup>-</sup>, wherein n is an integer of 1, 2, or 3, x is a number indicating the relative ratio between compound and acid (and may be a fraction), and Y is an anion, such as Cl<sup>-</sup>, Br<sup>-</sup>, I<sup>-</sup>, HSO<sub>4</sub><sup>-</sup>, SO<sub>4</sub><sup>2-</sup>, NO<sub>3</sub><sup>-</sup>, HCOO<sup>-</sup>, CH<sub>3</sub>COO<sup>-</sup>, HCO<sub>3</sub><sup>-</sup>, CO<sub>3</sub><sup>2-</sup>, H<sub>2</sub>PO<sub>4</sub><sup>-</sup>, HPO<sub>4</sub><sup>2-</sup>, PO<sub>4</sub><sup>3-</sup>, SCN<sup>-</sup>, BF<sub>4</sub><sup>-</sup>, ClO<sub>4</sub><sup>-</sup>, SSO<sub>3</sub><sup>-</sup>, CH<sub>3</sub>SO<sub>3</sub><sup>-</sup>, CH<sub>3</sub>C<sub>6</sub>H<sub>4</sub>SO<sub>3</sub><sup>-</sup>, SO<sub>3</sub><sup>2-</sup>, BrO<sub>3</sub><sup>-</sup>, IO<sub>3</sub><sup>-</sup>, ClO<sub>3</sub><sup>-</sup>, or the like. Examples of suitable morpholine acid salt compounds include

(1) 4-(2-chloroethyl) morpholine hydrochloride (Aldrich C4,220-3), of the formula:



63

(2) 4-morpholine ethane sulfonic acid (Aldrich 16,373-2), of the formula:



(3) 4-morpholine propane sulfonic acid (Aldrich 16,377-5), of the formula:



(4) 2-hydroxy morpholine propane sulfonic acid (Aldrich 28,481-5), of the formula:



(5) [N-(aminoiminomethyl)-4-morpholine carboximidamide] hydrochloride (Aldrich 27,861-0), of the formula:



(6) 4-morpholine carbodithioic acid compound with morpholine (Aldrich 32,318-7), of the formula:



(7) 2,5-dimethyl-4-(morpholinomethyl) phenol hydrochloride monohydrate (Aldrich 18,671-6), of the formula:



64

(8) 2-methoxy-4-morpholino benzene diazonium chloride, zinc chloride (Aldrich M1,680-6), of the formula:



15 (9) 1-cyclohexyl-3-(2-morpholinoethyl) carbodiimide metho-p-toluene sulfonate (Aldrich C10,640-2), of the formula:



20 (10) hemicholinium-3[2,2'-(4,4'-biphenylene) bis(2-hydroxy-4,4-dimethyl morpholinium bromide) (Aldrich H30,3), of the formula:



25 (11) hemicholinium-15[4,4-dimethyl-2-hydroxy-2-phenyl morpholinium bromide] (Aldrich 11,603-3), of the formula:



30 and the like.

Also suitable as antistatic agents are thiazole, thiazolidine, and thiadiazole acid salt compounds, of the general formulae



wherein R<sub>1</sub>, R<sub>2</sub>, R<sub>3</sub>, R<sub>4</sub>, R<sub>5</sub>, R<sub>6</sub>, and R<sub>7</sub> each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R<sub>1</sub>, R<sub>2</sub>, R<sub>3</sub>, R<sub>4</sub>, R<sub>5</sub>, R<sub>6</sub>, R<sub>7</sub>, R<sub>8</sub>, and R<sub>9</sub> can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds are in acid salt form, wherein they are associated with a compound of the general formula xH<sub>n</sub>Y<sub>n</sub><sup>-</sup>, wherein n is an integer of 1, 2, or 3, x is a number indicating the relative ratio between compound and acid (and may be a fraction), and Y is an anion, such as Cl<sup>-</sup>, Br<sup>-</sup>, I<sup>-</sup>, HSO<sub>4</sub><sup>2-</sup>, SO<sub>4</sub><sup>2-</sup>, NO<sub>3</sub><sup>-</sup>, HCOO<sup>-</sup>, CH<sub>3</sub>COO<sup>-</sup>, HCO<sub>3</sub><sup>-</sup>, CO<sub>3</sub><sup>2-</sup>, H<sub>2</sub>PO<sub>4</sub><sup>-</sup>, HPO<sub>4</sub><sup>2-</sup>, PO<sub>4</sub><sup>3-</sup>, SCN<sup>-</sup>, BF<sub>4</sub><sup>-</sup>, ClO<sub>4</sub><sup>-</sup>, SSO<sub>3</sub><sup>-</sup>, CH<sub>3</sub>SO<sub>3</sub><sup>-</sup>, CH<sub>3</sub>C<sub>6</sub>H<sub>4</sub>SO<sub>3</sub><sup>-</sup>, SO<sub>3</sub><sup>2-</sup>, BrO<sub>3</sub><sup>-</sup>, IO<sub>3</sub><sup>-</sup>, ClO<sub>3</sub><sup>-</sup>, or the like. Examples of suitable thiazole, thiazolidine, and thiadiazole acid salt compounds include

(1) 2-amino-4,5-dimethyl thiazole hydrochloride (Aldrich 17,440-8), of the formula:



(2) 2-amino 4-imino-2-thiazoline hydrochloride (Aldrich 13,318-3), of the formula:



10 (3) 2-amino-2-thiazoline hydrochloride (Aldrich 26,372-9), of the formula:



20 (4) 2-amino-5-bromothiazole monohydrobromide (Aldrich 12,802-3), of the formula:



25 (5) 5-amino-3-methyl isothiazole hydrochloride (Aldrich 15,564-0), of the formula:



35 (6) 2,2,5,5-tetramethyl-4-thiazolidine carboxylic acid hydrochloride hemihydrate (Aldrich P100-4), of the formula:



45 (7) 3-methyl-2-benzothiazolinone hydrazone hydrochloride hydrate (Aldrich 12,973-9), of the formula:



50 (8) 5-amino-2-methylbenzothiazole dihydrochloride (Aldrich A6,330-9), of the formula:



(9) 2,4-diamino-5-phenyl thiazole monohydrobromide (Aldrich D2,320-3), of the formula:



(10) 2-amino-4-phenyl thiazole hydrobromide monohydrate (Aldrich A7,500-5), of the formula:



(11) 2-(tritylaminio)- $\alpha$ -(methoxyimino)-4-thiazole acetic acid hydrochloride (Aldrich 28,018-6), of the formula:



(12) (2,3,5,6-tetrahydro-6-phenylimidazo [2,1-b] thiazole hydrochloride (Aldrich 19,613-4; 19614-2), of the formula:



and the like.

Also suitable as antistatic agents are phenothiazine acid salt compounds, of the general formula



wherein R<sub>1</sub>, R<sub>2</sub>, R<sub>3</sub>, R<sub>4</sub>, R<sub>5</sub>, R<sub>6</sub>, R<sub>7</sub>, R<sub>8</sub>, and R<sub>9</sub> each, independently of one another, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably

with from about 7 to about 31 carbon atoms and more preferably with from about 7 to about 20 carbon atoms, substituted arylalkyl groups, preferably with from about 7 to about 32 carbon atoms and more preferably with from about

5 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein  
10 two or more of R<sub>1</sub>, R<sub>2</sub>, R<sub>3</sub>, R<sub>4</sub>, R<sub>5</sub>, R<sub>6</sub>, R<sub>7</sub>, R<sub>8</sub>, and R<sub>9</sub> can be joined together to form a ring, and wherein the substituents on the substituted alkyl groups, substituted aryl groups, and substituted arylalkyl groups can be (but are not limited to)  
15 hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible,  
20 such as a double bond between one of the ring carbon atoms and another atom, such as carbon, oxygen, or the like. These compounds are in acid salt form, wherein they are associated with a compound of the general formula xH<sub>n</sub>Y<sub>n</sub><sup>-</sup>, wherein n is an integer of 1, 2, or 3, x is a number indicating the relative ratio between compound and acid (and may be a fraction), and Y is an anion, such as Cl<sup>-</sup>, Br<sup>-</sup>, I<sup>-</sup>, HSO<sub>4</sub><sup>2-</sup>, SO<sub>4</sub><sup>2-</sup>, NO<sub>3</sub><sup>-</sup>, HCOO<sup>-</sup>, CH<sub>3</sub>COO<sup>-</sup>, HCO<sub>3</sub><sup>-</sup>, CO<sub>3</sub><sup>2-</sup>, H<sub>2</sub>PO<sub>4</sub><sup>-</sup>, HPO<sub>4</sub><sup>2-</sup>, PO<sub>4</sub><sup>3-</sup>, SCN<sup>-</sup>, BF<sub>4</sub><sup>-</sup>, ClO<sub>4</sub><sup>-</sup>, SSO<sub>3</sub><sup>-</sup>, CH<sub>3</sub>SO<sub>3</sub><sup>-</sup>, CH<sub>3</sub>C<sub>6</sub>H<sub>4</sub>SO<sub>3</sub><sup>-</sup>, SO<sub>3</sub><sup>2-</sup>, BrO<sub>3</sub><sup>-</sup>, IO<sub>3</sub><sup>-</sup>, ClO<sub>3</sub><sup>-</sup>, or the like.  
25  
30  
35  
40 Examples of suitable phenothiazine acid salt compounds include

(1) trifluoroperazine dihydrochloride (Aldrich 28,388-6), of the formula:



(2) thioridazine hydrochloride (Aldrich 25,770-2), of the formula:



(3) ( $\pm$ )-promethazine hydrochloride (Aldrich 28,411-4), of the formula:



(4) ethopropazine hydrochloride (Aldrich 28,583-8), of the formula:



(5) chlorpromazine hydrochloride (Aldrich 28,537-4), of the formula:



and the like.

Preferred antistatic agents are monomeric, although dimeric, trimeric, oligomeric, and polymeric antistatic agents can also be employed.

If an optional overcoating layer is used on top of the softenable layer to improve abrasion resistance and if solvent softening is employed to effect migration of the migration marking material through the softenable material, the overcoating layer should be permeable to the vapor of the solvent used and additional vapor treatment time should be allowed so that the solvent vapor can soften the softenable layer sufficiently to allow the light-exposed migration marking material to migrate towards the substrate in image configuration. Solvent permeability is unnecessary for an overcoating layer if heat is employed to soften the softenable layer sufficiently to allow the exposed migration marking material to migrate towards the substrate in image configuration.

Further information concerning the structure, materials, and preparation of migration imaging members is disclosed in U.S. Pat. No. 3,975,195, U.S. Pat. No. 3,909,262, U.S. Pat. No. 4,536,457, U.S. Pat. No. 4,536,458, U.S. Pat. No. 4,013,462, U.S. Pat. No. 4,883,731, U.S. Pat. No. 4,123,283, U.S. Pat. No. 4,853,307, U.S. Pat. No. 4,880,715, U.S. application Ser. No. 590,959 (abandoned, filed Oct. 31, 1966), U.S. application Ser. No. 695,214 (abandoned, filed Jan. 2, 1968), U.S. application Ser. No. 000,172 (abandoned, filed Jan. 2, 1970), and P. S. Vincett, G. J. Kovacs, M. C. Tam, A. L. Pundsack, and P. H. Soden, *Migration Imaging Mechanisms, Exploitation, and Future Prospects of Unique Photographic Technologies, XDM and AMEN*, Journal of Imaging Science 30 (4) July/August, pp. 183-191 (1986), the disclosures of each of which are totally incorporated herein by reference.

If desired, one or more additional softenable layers containing migration marking material can be employed in the

imaging member, as disclosed in copending application U.S. Ser. No. 08/353,461, entitled "Improved Migration Imaging Members", the disclosure of which is totally incorporated herein by reference. The additional softenable layer or layer 5 can be applied to the imaging member by any suitable or desired method, such as by lamination, wherein the second softenable layer is initially coated onto a second substrate, followed by placing the surface of the second softenable layer in contact with the surface of the first softenable layer 10 and applying heat and pressure, and subsequently removing the second substrate from the second softenable layer now adhering to the first softenable layer. In preferred embodiments, the lamination process takes place in a vacuum environment, as disclosed in copending application Ser. No. 08/432,747, entitled "Process and Apparatus for Manufacturing Migration Imaging Members", the disclosure of which is totally incorporated herein by reference.

The migration imaging member of the present invention is imaged and developed to provide an imagewise pattern on the member. The imaged member can be used as an information recording and storage medium, for viewing and as a duplicating film, as a mask for exposing photosensitive lithographic printing plates, as a xeroprinting master in a xeroprinting process, or for any other desired purpose.

25 The process for imaging an imaging member of the present invention as shown schematically in FIG. 1 is illustrated schematically in FIGS. 2, 3, 4, 5, and 6. FIGS. 2 through 6 illustrate schematically a migration imaging member comprising a conductive substrate layer 22 that is connected to a reference potential such as a ground, and a softenable layer 26 comprising softenable material 27, migration marking material 28, infrared or red light sensitive pigment particles 24, and optional first charge transport material 30. As illustrated in FIG. 2, the member is uniformly charged in the dark to either polarity (negative charging is illustrated in FIG. 2) by a charging means 29 such as a corona charging apparatus.

As illustrated schematically in FIG. 3, the charged member is first exposed imagewise to infrared or red light radiation 31. The wavelength of the infrared or red light radiation used is preferably selected to be in the region where the infrared or red-light sensitive pigment 24 exhibits maximum optical absorption and maximum photosensitivity. Infrared or red light radiation 31 passes through the non-absorbing migration marking material 28 (which is selected to be substantially insensitive to the infrared or red light radiation wavelength used in this step) and exposes the infrared or red light sensitive pigment particles 24 in the softenable layer. Absorption of infrared or red light radiation 45 by the infrared or red light sensitive pigment results in substantial photodischarge in the exposed areas. Thus the areas that are exposed to infrared radiation become substantially discharged.

50 As illustrated schematically in FIG. 4, the charged member is subsequently exposed uniformly to activating radiation 32 at a wavelength to which the migration marking material 28 is sensitive. For example, when the migration marking material is selenium particles, blue or green light can be used for uniform exposure. Uniform exposure to radiation 32 results in absorption of radiation by the migration marking material 28. In charged areas of the imaging member 35, the migration marking particles 28a acquire a negative charge as ejected holes (positive charges) discharge the surface charges, resulting in an electric field between the 55 migration marking particles and the substrate. Areas 37 of the imaging member that have been substantially discharged by prior infrared or red light exposure are no longer sensi-

tive, and the migration marking particles **28b** in these areas acquire no or very little charge. The wavelength of the uniform light radiation is preferably selected to be in the region where the infrared or red-light sensitive pigments in the softenable layer exhibit maximum light transmission and where the migration marking particles **28** exhibit maximum light absorption. Thus, in areas of the imaging member which are still charged, the migration marking particles **28a** acquire a negative charge as ejected holes (positive charges) transport through the softenable layer to the substrate. Areas **37** of the imaging member that have been substantially discharged by prior infrared or red light exposure are no longer light sensitive, and the migration marking particles **28b** in these areas acquire no or very little charge.

It is important to emphasize that in general, the step of imagewise exposing the member to infrared or red light radiation and the step of uniformly exposing the member to radiation at a wavelength to which the migration marking material is sensitive can take place in any order. When the member is first imagewise exposed to infrared or red light radiation as illustrated in FIG. 3 and subsequently uniformly exposed to radiation to which the migration marking material is sensitive as illustrated in FIG. 4, the process proceeds as described with respect to said Figures. When the member is first uniformly exposed to radiation to which the migration marking material is sensitive and subsequently imagewise exposed to infrared or red light radiation, the process proceeds as described with respect to FIGS. 5, 6, and 7.

As illustrated schematically in FIG. 5, the charged member illustrated schematically in FIG. 2 is first exposed uniformly to activating radiation **32** at a wavelength to which the migration marking material **28** is sensitive. For example, when the migration marking material is selenium particles, blue or green light can be used for uniform exposure. Uniform exposure to radiation **32** results in absorption of radiation by the migration marking material **28**. The migration marking particles **28** acquire a negative charge as ejected holes (positive charges) discharge the surface negative charges.

As illustrated schematically in FIG. 6, the charged member is subsequently exposed imagewise to infrared or red light radiation **31**. Infrared or red light radiation **31** passes through the non-absorbing migration marking material **28** (which is selected to be insensitive to the infrared or red light radiation wavelength used in this step) and exposes the infrared or red light sensitive pigment particles **24** in the softenable layer, thereby discharging the migration marking particles **28b** in area **37** that are exposed to infrared or red light radiation and leaving the migration marking particles **28a** charged in areas **35** not exposed to infrared or red light radiation.

As illustrated schematically in FIG. 7, subsequent to formation of a charge image pattern, the imaging member is developed by causing the softenable material to soften by any suitable means (in FIG. 7, by uniform application of heat energy **33** to the member). The heat development temperature and time depend upon factors such as how the heat energy is applied (e.g. conduction, radiation, convection, and the like), the melt viscosity of the softenable layer, thickness of the softenable layer, the amount of heat energy, and the like. For example, at a temperature of 110° C. to about 130° C., heat need only be applied for a few seconds. For lower temperatures, more heating time can be required. When the heat is applied, the softenable material **27** decreases in viscosity, thereby decreasing its resistance to migration of the marking material **28** through the softenable layer **26**. As shown in FIG. 7, in areas **35** of the imaging

member, wherein the migration marking particles **28a** have a substantial net charge, upon softening of the softenable material **27**, the net charge causes the charged marking material to migrate in image configuration towards the conductive layer **22** and disperse or agglomerate in the softenable layer **26**, resulting in a  $D_{min}$  area. The uncharged migration marking particles **28b** in areas **37** of the imaging member remain essentially neutral and uncharged. Thus, in the absence of migration force, the unexposed migration marking particles remain substantially in their original position in softenable layer **26**, resulting in a  $D_{max}$  area.

If desired, solvent vapor development can be substituted for heat development. Vapor development of migration imaging members is well known in the art. Generally, if solvent vapor softening is utilized, the solvent vapor exposure time depends upon factors such as the solubility of the softenable layers in the solvent, the type of solvent vapor, the ambient temperature, the concentration of the solvent vapors, and the like.

The application of either heat, or solvent vapors, or combinations thereof, or any other suitable means should be sufficient to decrease the resistance of the softenable material **27** of softenable layer **26** to allow migration of the migration marking material **28** through softenable layer **26** in imagewise configuration. With heat development, satisfactory results can be achieved by heating the imaging member to a temperature of about 100° C. to about 130° C. for only a few seconds when the uncoated softenable layer contain an 80/20 mole percent copolymer of styrene and hexylmethacrylate having an intrinsic viscosity of 0.179 dl/gm and N,N'-diphenyl-N,N'-bis(3"-methylphenyl)-(1,1'-biphenyl)-4,4'-diamine. The test for a satisfactory combination of time and temperature is to maximize optical contrast density. With vapor development, satisfactory results can be achieved by exposing the imaging member to the vapor of toluene for between about 4 seconds and about 60 seconds at a solvent vapor partial pressure of between about 5 millimeters and 30 millimeters of mercury when the uncoated softenable layer contain an 80/20 mole percent copolymer of styrene and hexylmethacrylate having an intrinsic viscosity of 0.179 dl/gm and N,N'-diphenyl-N,N'-bis(3"-methylphenyl)-(1,1'-biphenyl)-4,4'-diamine.

The imaging member illustrated in FIGS. 2 through 7 is shown without any optional layers such as those illustrated in FIG. 1. If desired, alternative imaging member embodiments, such as those employing any or all of the optional layers illustrated in FIG. 1, can also be employed.

Specific embodiments of the invention will now be described in detail. These examples are intended to be illustrative, and the invention is not limited to the materials, conditions, or process parameters set forth in these embodiments. All parts and percentages are by weight unless otherwise indicated.

#### EXAMPLE I

##### A

Three migration imaging members having a single softenable layer were prepared as follows. A solution for the softenable layers was prepared by dissolving about 497.3 grams of a terpolymer of styrene/ethylacrylate/acrylic acid (prepared as disclosed in U.S. Pat. No. 4,853,307, the disclosure of which is totally incorporated herein by reference) and about 24 grams of X-metal-free phthalocyanine (prepared as described in U.S. Pat. No. 3,357,989 (Byrne et al.), the disclosure of which is totally incorporated by

reference) in about 1478.7 grams of toluene. The solution was pumped through a M110 Y laboratory Microfluidizer, obtained from Microfluidics Corporation, Newton, Mass., for a total of 3 passes at a liquid pressure of 12,000 pounds per square inch, with water cooling at 10° C. to reduce the particle size of the pigment, followed by filtering the solution by positive nitrogen pressure up to 30 kPa through a Pall 1.0 micron filter cartridge. The resulting solution was coated by a solvent extrusion technique onto three 4 mil thick polyester substrates (Melinex 442, obtained from Imperial Chemical Industries (ICI), aluminized to 50 percent light transmission) at a coating speed of 8 feet per minute, and the deposited softenable layers were allowed to dry at about 115° C. for about 2 minutes, resulting in dried softenable layers with thicknesses of about 2 microns. The temperature of the softenable layers was then raised to about 115° C. to lower the viscosity of the exposed surfaces of the softenable layers to about  $5 \times 10^3$  poises in preparation for the deposition of marking material. Thin layers of particulate vitreous selenium were then applied by vacuum deposition in a vacuum chamber maintained at a vacuum of about  $4 \times 10^{-4}$  Torr. The imaging members were then rapidly chilled to room temperature. Reddish monolayers of selenium particles having an average diameter of about 0.3 micron embedded about 0.05 to 0.1 micron below the surfaces of the copolymer layers were formed.

## B

Three additional imaging members were prepared as described above in Paragraph A except that the solution for the softenable layers was prepared by dissolving about 84 parts by weight of a terpolymer of styrene/ethylacrylate/acrylic acid and about 16 parts by weight of N,N'-diphenyl-N,N'-bis(3"-methylphenyl)-(1,1'-biphenyl)-4,4'-diamine (prepared as disclosed in U.S. Pat. No. 4,265,990, the disclosure of which is totally incorporated herein by reference) in about 450 parts by weight of toluene. N,N'-diphenyl-N,N'-bis(3"-methylphenyl)-(1,1'-biphenyl)-4,4'-diamine is a charge transport material capable of transporting positive charges (holes). The resulting solution was coated by a solvent extrusion technique onto three 3 mil thick polyester substrates (Melinex 442, obtained from Imperial Chemical Industries (ICI), aluminized to 20 percent light transmission), and the deposited softenable layers were allowed to dry at about 115° C. for about 2 minutes, resulting in dried softenable layers with thicknesses of about 4 microns. These second imaging members were wound onto 1 inch diameter cardboard tube laminating cores. The first imaging members prepared in Paragraph A were also wound onto 1 inch diameter cardboard tube laminating cores. Three migration imaging members, each having one softenable layer prepared as described in Paragraph A and one softenable layer prepared as described in Paragraph B, were prepared as follows. The two rolls of imaging member sheets were mounted on the support brackets in an AGFA ADL laminator. The normal operation of this laminator is to have two rolls of laminating material mounted on support brackets. The film is threaded and joined. An item, such as a poster or placemat, for instance, can be placed between the two sheets and run through pinch and drive rollers, resulting in placement of a protective overcoat on both sides of the item. In this instance, the rolls of imaging member were mounted on the support brackets which ordinarily bear the rolls of protective coating material. The imaging members were threaded and joined so that the softenable layer of the first member was in contact with the softenable layer of the

second member. Sections of the "sandwich" thus formed were then fed through the laminator at a temperature of 100° C. After the "sandwich" had passed through the laminator and was cut from the machine, it was left to cool for a few minutes, after which the substrate of the imaging member prepared in Paragraph B was carefully peeled apart from the softenable layer, resulting in formation of a single migration imaging member having two softenable layers on the aluminized Mylar® substrate of Paragraph A.

10

## C

Sections of the migration imaging members prepared as described in Paragraph B were placed on a charge table and grounded with copper tape. To establish film ground prior to charging. With all room lights off, the imaging member sections were negatively charged with a corotron, and then were removed from the table and exposed imagewise to infrared light of 773 nanometers through a silver halide mask for a period of 10 seconds. Subsequent to exposure to infrared light in an image pattern, the imaging member sections were placed back on the charge table and exposed uniformly to blue light of 490 nanometers for a period of 10 seconds. The imaging member sections were then developed by subjecting them to a temperature of 115° C. for a period of 5 seconds using a small aluminum heating block in contact with the polyester substrate. The optical densities of the  $D_{min}$  and  $D_{max}$  areas were then measured using a MacBeth TR927 densitometer. The background values attributable to the substrate were not subtracted from the values shown in the table. The blue setting corresponds to a Wratten No. 47 filter and the ultraviolet setting corresponds to a Wratten No. 18A filter.

35

## D

For comparison purposes, another imaging member was prepared by preparing an imaging member as described in Paragraph B except that both the first and second softenable layers contained 84 percent by weight of the softenable material and 16 percent by weight of the charge transport material, and a separate infrared-sensitive layer was applied to the surface of the two softenable layers by the following procedure. A pigment dispersion was prepared by ball milling for 24 hours a mixture comprising 10.6 parts by weight solids in a solvent (wherein the solvent comprised 40 percent by weight 2-propanol and 60 percent by weight deionized water), wherein the solids comprised 20 percent by weight X-metal-free phthalocyanine and 80 percent by weight of a styrene-butyl methacrylate copolymer (ICI Neocryl A622). The resulting dispersion was hand coated onto the top softenable layers of the migration imaging members with a #5 Meyer rod, followed by drying the deposited infrared-sensitive layers at 50° C. for 1 minute by contacting the polyester substrates to an aluminum heating block. This imaging member was imaged as follows. The surface of the member was uniformly positively charged with a corona charging device and subsequently exposed by placing a test pattern mask comprising a silver halide image in contact with the imaging member and exposing the member to infrared light of 773 nanometers through the mask for a period of 20 seconds. The exposed member was subsequently uniformly exposed to 490 nanometer light for a period of 10 seconds and thereafter uniformly negatively recharged with a corona charging device. The imaging member was then developed by subjecting it to a temperature of 105° C. for a period of 5 seconds using a small aluminum heating block in contact with the polyester sub-

strate. The optical densities of the  $D_{min}$  and  $D_{max}$  areas were then measured using a MacBeth TR927 densitometer. The background values attributable to the substrate were not subtracted from the values shown in the table. The blue setting corresponds to a Wratten No. 47 filter and the ultraviolet setting corresponds to a Wratten No. 18A filter.

Optical densities for the infrared-sensitive imaging members were as follows:

| Imaging | Optical Density (blue) |           |           | Optical Density (ultraviolet) |           |           |
|---------|------------------------|-----------|-----------|-------------------------------|-----------|-----------|
|         | Member                 | $D_{min}$ | $D_{max}$ | $\Delta O.D.$                 | $D_{min}$ | $D_{max}$ |
| B1      | 1.42                   | 2.41      | 0.99      | 1.84                          | 2.64      | 0.80      |
| B2      | 1.39                   | 2.44      | 1.05      | 1.81                          | 2.72      | 0.91      |
| B3      | 1.39                   | 2.37      | 0.98      | 1.77                          | 2.67      | 0.90      |
| D1      | 0.92                   | 1.80      | 0.88      | 2.06                          | 2.80      | 0.74      |
| D2      | 1.02                   | 2.89      | 1.87      | 2.48                          | 4.10      | 1.62      |

As the data indicate, the imaging members prepared as described in Paragraph B exhibited significantly lower  $D_{min}$  values in the ultraviolet range compared to the imaging members prepared as described in Paragraph D. In addition, the optical contrast densities were improved in both the blue and ultraviolet regions for the imaging members prepared as described in Paragraph B as compared to the imaging member prepared as described in Paragraph D.

The imaging procedures described above in Paragraphs C and D were repeated, except that the imaging members were first exposed uniformly to blue light and then exposed to infrared light in an imagewise pattern. Similar results were observed.

Other embodiments and modifications of the present invention may occur to those skilled in the art subsequent to a review of the information presented herein; these embodiments and modifications, as well as equivalents thereof, are also included within the scope of this invention.

What is claimed is:

1. A migration imaging member comprising a substrate and a softenable layer, said softenable layer comprising a softenable material, a pigment predominantly sensitive to infrared or red light radiation dispersed uniformly throughout the softenable layer, and a migration marking material predominantly sensitive to radiation at a wavelength other than that to which the infrared or red light radiation sensitive pigment is sensitive, wherein the migration marking material is present in the softenable layer as a monolayer of particles situated at or near the surface of the softenable layer spaced from the substrate.

2. A migration imaging member according to claim 1 wherein the softenable layer is substantially free of a charge transport material.

3. A migration imaging member according to claim 1 wherein the softenable layer also contains a charge transport material.

4. A migration imaging member according to claim 1 wherein the migration marking material is selenium.

5. A migration imaging member according to claim 1 wherein the pigment sensitive to infrared or red light radiation is selected from the group consisting of benzimidazole perylene, dibromoanthranthrone, trigonal selenium, beta-metal free phthalocyanine, X-metal free phthalocyanine, vanadyl phthalocyanine, chloroindium phthalocyanine, titanyl phthalocyanine, chloroaluminum phthalocyanine, copper phthalocyanine, magnesium phthalocyanine, and mixtures thereof.

6. A migration imaging member according to claim 1 wherein the pigment sensitive to infrared or red light radiation is X-metal free phthalocyanine.

7. A migration imaging member according to claim 1 wherein the softenable material is a styrene/ethyl acrylate/acrylic acid terpolymer.

8. A migration imaging member according to claim 1 wherein the imaging member also comprises a second softenable layer containing a second softenable material, a second migration marking material, and an optional charge transport material.

9. A migration imaging member according to claim 1 wherein the pigment sensitive to infrared or red light radiation is present in an amount of from about 10 to about 60 percent by weight of the softenable layer.

10. A migration imaging member according to claim 1 wherein the pigment sensitive to infrared or red light radiation is present in an amount of from about 10 to about 20 percent by weight of the softenable layer.

11. A migration imaging process which comprises the steps of (A) providing a migration imaging member comprising a substrate and a softenable layer, said softenable layer comprising a softenable material, a pigment predominantly sensitive to infrared or red light radiation dispersed uniformly throughout the softenable layer, and a migration marking material predominantly sensitive to radiation at a wavelength other than that to which the infrared or red light radiation sensitive pigment is sensitive, wherein the migration marking material is present in the softenable layer as a monolayer of particles situated at or near the surface of the softenable layer spaced from the substrate; (B) uniformly charging the imaging member; (C) subsequent to step B, exposing the charged imaging member to infrared or red light radiation at a wavelength to which the infrared or red light radiation sensitive pigment is sensitive in an imagewise pattern, thereby forming an electrostatic latent image on the imaging member; (D) subsequent to step B, uniformly exposing the imaging member to activating radiation at a wavelength to which the migration marking material is sensitive; and (E) subsequent to steps C and D, causing the softenable material to soften, thereby enabling the migration marking material to migrate through the softenable material toward the substrate in an imagewise pattern.

12. A migration imaging process according to claim 11 wherein the softenable layer is substantially free of a charge transport material.

13. A migration imaging process according to claim 11 wherein the softenable layer also contains a charge transport material.

14. A migration imaging process according to claim 11 wherein the migration marking material is selenium.

15. A migration imaging process according to claim 11 wherein the pigment sensitive to infrared or red light radiation is selected from the group consisting of benzimidazole perylene, dibromoanthranthrone, trigonal selenium, beta-metal free phthalocyanine, X-metal free phthalocyanine, vanadyl phthalocyanine, chloroindium phthalocyanine, titanyl phthalocyanine, chloroaluminum phthalocyanine, copper phthalocyanine, magnesium phthalocyanine, and mixtures thereof.

16. A migration imaging process according to claim 11 wherein the pigment sensitive to infrared or red light radiation is X-metal free phthalocyanine.

17. A migration imaging process according to claim 11 wherein the softenable material is a styrene/ethyl acrylate/acrylic acid terpolymer.

18. A migration imaging process according to claim 11 wherein the imaging member also comprises a second softenable layer containing a second softenable material, a second migration marking material, and an optional charge transport material.

**19.** A migration imaging process according to claim 11 wherein the pigment sensitive to infrared or red light radiation is present in an amount of from about 10 to about 60 percent by weight of the softenable layer.

**20.** A migration imaging process according to claim 11 wherein the pigment sensitive to infrared or red light radiation is present in an amount of from about 10 to about 20 percent by weight of the softenable layer.

**21.** A migration imaging process according to claim 11

wherein the softenable material is caused to soften by the application of heat.

**22.** A migration imaging process according to claim 11 wherein step (C) takes place before step (D).

**23.** A migration imaging process according to claim 11 wherein step (D) takes place before step (C).

\* \* \* \* \*